



US010828884B2

(12) **United States Patent**  
Merka et al.

(10) **Patent No.:** US 10,828,884 B2  
(45) **Date of Patent:** Nov. 10, 2020

(54) **LITHOGRAPHIC PRINTING PLATE PRECURSORS AND METHOD OF USE**

(71) Applicant: **Eastman Kodak Company**, Rochester, NY (US)

(72) Inventors: **Oliver Merka**, Gottingen (DE); **Jan-Phillip Kemmling**, Bilshausen (DE); **Oliver Richard Blum**, Bovenden (DE); **Benedikt Uhl**, Ulm (DE)

(73) Assignee: **EASTMAN KODAK COMPANY**, Rochester, NY (US)

(\*) Notice: Subject to any disclaimer, the term of this patent is extended or adjusted under 35 U.S.C. 154(b) by 420 days.

(21) Appl. No.: **15/447,651**

(22) Filed: **Mar. 2, 2017**

(65) **Prior Publication Data**

US 2018/0250925 A1 Sep. 6, 2018

(51) **Int. Cl.**

**B4IN 1/14** (2006.01)  
**B4IN 1/22** (2006.01)

(Continued)

(52) **U.S. Cl.**

CPC ..... **B41C 1/1008** (2013.01); **B4IN 1/083** (2013.01); **B4IN 1/14** (2013.01); **B4IN 1/22** (2013.01);

(Continued)

(58) **Field of Classification Search**

None

See application file for complete search history.

(56)

**References Cited**

U.S. PATENT DOCUMENTS

4,566,952 A 1/1986 Sprintschnik et al.  
8,783,179 B2 7/2014 Kurokawa et al.

(Continued)

FOREIGN PATENT DOCUMENTS

EP 0316240 A1 5/1989  
EP 1642745 A2 4/2006

(Continued)

*Primary Examiner* — Joshua D Zimmerman

(57)

**ABSTRACT**

Lithographic printing plate precursors are prepared with a unique substrate and one or more radiation-sensitive imageable layers. The substrate is prepared by two separate anodizing processes to provide an inner aluminum oxide layer having an average dry thickness ( $T_i$ ) of 650-3,000 nm and a multiplicity of inner micropores having an average inner micropore diameter ( $D_i$ ) of  $\leq 15$  nm. A formed outer aluminum oxide layer comprises a multiplicity of outer micropores having an average outer micropore diameter ( $D_o$ ) of 15-30 nm; an average dry thickness ( $T_o$ ) of 130-650 nm; and a micropore density ( $C_o$ ) of 500-3,000 micropores/ $\mu\text{m}^2$ . The ratio of  $D_o$  to  $D_i$  is greater than 1.1:1, and  $D_o$  in nanometers and the outer aluminum oxide layer micropore density ( $C_o$ ) in micropores/ $\mu\text{m}^2$ , are further defined by the outer aluminum oxide layer porosity ( $P_o$ ) according to the following equation:

$$0.3 \leq P_o \leq 0.8$$

where  $P_o$  is  $3.14(C_o)(D_o^2)/4,000,000$ .

**13 Claims, 1 Drawing Sheet**



(51) **Int. Cl.**  
*B41C 1/10* (2006.01)  
*C25D 11/16* (2006.01)  
*B41N 3/03* (2006.01)  
*C25D 11/08* (2006.01)  
*B41N 1/08* (2006.01)  
*C25D 11/12* (2006.01)

(52) **U.S. Cl.**  
CPC ..... *B41N 3/034* (2013.01); *C25D 11/08* (2013.01); *C25D 11/12* (2013.01); *C25D 11/16* (2013.01); *B41C 2210/04* (2013.01); *B41C 2210/08* (2013.01); *B41N 3/036* (2013.01)

(56) **References Cited**

U.S. PATENT DOCUMENTS

2008/0003411 A1 1/2008 Hunter et al.  
2011/0265673 A1 11/2011 Tagawa et al.  
2012/0192742 A1 8/2012 Kurokawa et al.  
2013/0052582 A1 2/2013 Hayashi  
2014/0047993 A1 2/2014 Hauck et al.  
2014/0326151 A1 11/2014 Namba et al.  
2015/0135979 A1 \* 5/2015 Tagawa ..... C25F 3/04  
101/454

FOREIGN PATENT DOCUMENTS

EP 2353882 A1 8/2011  
EP 2520439 A1 11/2012  
JP 2005254638 A \* 9/2005

\* cited by examiner



LITHOGRAPHIC PRINTING PLATE  
PRECURSORS AND METHOD OF USE

## FIELD OF THE INVENTION

This invention relates to lithographic printing plate precursors comprising an inventive aluminum-containing substrate that has been prepared using two separate anodizing processes to provide different aluminum oxide layers with different structural properties. This invention also relates to a method for imaging and processing such lithographic printing plate precursors to provide lithographic printing plates; and it further relates to a method of making such precursors using two anodizing processes.

## BACKGROUND OF THE INVENTION

In lithographic printing, lithographic ink receptive regions, known as image areas, are generated on a hydrophilic planar surface of a substrate. When the printing plate surface is moistened with water and a lithographic printing ink is applied, hydrophilic regions retain the water and repel the lithographic printing ink, and the lithographic ink receptive image regions accept the lithographic printing ink and repel the water. The lithographic printing ink is transferred from the lithographic printing plate to the surface of a material upon which the image is to be reproduced, perhaps with the use of a blanket roller.

Imageable elements or lithographic printing plate precursors used to prepare lithographic printing plates typically comprise one or more radiation-sensitive imageable layers disposed on the outermost hydrophilic surface of the substrate. Such radiation-sensitive imageable layers comprise one or more radiation-sensitive components that can be dispersed together or within a polymeric binder material. Alternatively, a radiation-sensitive component can also serve as or form a polymeric binder material. Following imaging, either the exposed (imaged) regions or the non-exposed (non-imaged) regions of the one or more radiation-sensitive layers can be removed using a suitable developer, revealing the outermost hydrophilic surface of the substrate. If the exposed regions are removable, the lithographic printing plate precursor is considered positive-working. Conversely, if the non-exposed regions are removable, the lithographic printing plate precursor is considered negative-working.

Direct digital thermal imaging of lithographic printing plate precursors has become increasingly important in the printing industry in the last 30 years because of their stability to ambient light. Such precursors have been designed to be sensitive to imaging near-infrared radiation of at least 750 nm. However, other very useful lithographic printing plate precursors are still designed to be sensitive to digital imaging with UV or "violet" radiation of at least 250 nm.

Negative-working lithographic printing plate precursors useful to prepare lithographic printing plates typically comprise a negative-working radiation-sensitive imageable layer disposed over the hydrophilic surface of a substrate. Radiation-sensitive photopolymerizable compositions used in negative-working lithographic printing plate precursors typically comprise free-radically polymerizable components, one or more radiation absorbers, an initiator composition, and optionally one or more polymeric binders that are different from the other noted components.

In recent years, there has been an emphasis in the industry for simplification of the lithographic printing plate making process, including an omission of the pre-development

heating step (preheat) and carrying out development on-press (DOP) using a lithographic printing ink, fountain solution, or both, to remove unwanted (non-exposed) imageable layer materials on the lithographic printing plate precursors. Such negative-working lithographic printing plate precursors must be designed by balancing many features within the element structure in order to achieve optimal press life, on-press developability, and scratch resistance. It has not been an easy task to achieve high quality in all of these properties because what chemical composition or structural features may provide optimal level in one or two properties may cause a loss in another property.

Independently of the type of lithographic printing plate precursor, lithography has generally been carried out using a metal-containing substrate comprising aluminum or an aluminum-alloy of various metal compositions, for example containing up to 10 weight % of one or more of other metals known in the art for this purpose. The raw stock aluminum-containing material can be cleaned in a "pre-etch" process using a base or surfactant solution to remove oil, grease, and other contaminants on the planar surface of the raw stock aluminum-containing material. The cleaned planar surface is then generally roughed by electrochemical or mechanical graining, followed by a "post-etch" treatment to remove any contaminants ("smut") formed during the graining process. Further industrial details of the preparation of useful substrates for lithographic printing plate precursors are found in U.S. Patent Application Publication 2014/0047993 A1 (Hauck et al.).

After further rinsing, the planar surface of the aluminum-containing substrate is then anodized one or more times to provide an outermost hydrophilic aluminum oxide coating for abrasion resistance and other properties of the resulting lithographic printing plate precursor once one or more imageable layers have been formed thereon.

One or more anodizing processes are used in some known methods of making precursor substrates, for example, as described in U.S. Pat. No. 4,566,952 (Sprintzchnik et al.) and U.S. Pat. No. 8,783,179 (Kurokawa et al.), U.S. Patent Application Publications 2011/0265673 (Tagawa et al.), 2012/0192742 (Kurokawa et al.), 2014/0326151 (Namba et al.), and 2015/0135979 (Tagawa et al.), and EP 2,353,882A1 (Tagawa et al.).

In these known methods of making precursor substrates, sulfuric acid, phosphoric acid, or both sulfuric acid and phosphoric acid have been used as electrolytes in combination with various process parameters in order to produce one or more anodic (aluminum oxide) layers of specific structures and thus achieve specific properties in the resulting precursors. However, it has been found that lithographic printing plate precursors prepared according to these known methods are still unsatisfactory in one or more precursor properties such as scratch resistance, on-press developability, and press life.

Thus, there remains a need to balance the manufacturing conditions, especially during anodization, for negative-working lithographic printing plate precursors so that improved scratch resistance is achieved without sacrificing press life and on-press developability.

## SUMMARY OF THE INVENTION

The present invention provides a lithographic printing plate precursor comprising:

a substrate having a planar surface, and  
a radiation-sensitive imageable layer disposed over the planar surface of the substrate,

wherein the substrate comprises:

an aluminum-containing plate having a grained and etched planar surface;

an inner aluminum oxide layer disposed on the grained and etched planar surface, the inner aluminum oxide layer: having an average dry thickness ( $T_i$ ) of at least 650 nm and up to and including 3,000 nm; and comprising a multiplicity of inner micropores having an average inner micropore diameter ( $D_i$ ) of less than or equal to 15 nm;

an outer aluminum oxide layer disposed on the inner aluminum oxide layer, the outer aluminum oxide layer: comprising a multiplicity of outer micropores having an average outer micropore diameter ( $D_o$ ) of at least 15 nm and up to and including 30 nm; having an average dry thickness ( $T_o$ ) of at least 130 nm and up to and including 650 nm; and having a micropore density ( $C_o$ ) of at least 500 micropores/ $\mu\text{m}^2$  and up to and including 3,000 micropores/ $\mu\text{m}^2$ , wherein the ratio of the average outer micropore diameter ( $D_o$ ) to the average inner micropore diameter ( $D_i$ ) is greater than 1.1:1, and the average outer micropore diameter ( $D_o$ ) in nanometers and the micropore density ( $C_o$ ) in micropores/ $\mu\text{m}^2$ , are further constrained by the porosity ( $P_o$ ) of the outer aluminum oxide layer according to the following equation:

$$0.3 \leq P_o \leq 0.8$$

wherein  $P_o$  is defined as  $3.14(C_o)(D_o)^2/4,000,000$ ; and

optionally a hydrophilic layer comprising one or more hydrophilic polymers, which hydrophilic layer is disposed on the outer aluminum oxide layer at a dry coverage of at least 0.0002 g/m<sup>2</sup> and up to and including 0.1 g/m<sup>2</sup>.

In some embodiments of the present invention, the precursor is further defined, wherein:

the grained and etched planar surface of the aluminum-containing plate has been electrochemically grained and etched;

the radiation-sensitive imageable layer is a negative-working and on-press developable infrared radiation-sensitive imageable layer that is disposed on the electrochemically grained and etched planar surface, and comprises:

- (a) one or more free radically polymerizable components;
- (b) an initiator composition that provides free radicals upon exposure of the radiation-sensitive imageable layer to infrared radiation;
- (c) one or more infrared radiation absorbers; and
- (d) a particulate polymeric binder that is different from all of (a), (b), and (c);

the inner aluminum oxide layer has an average dry thickness ( $T_i$ ) of at least 700 nm and up to and including 1,500 nm;

the outer aluminum oxide layer has an average dry thickness ( $T_o$ ) of at least 130 nm and up to and including 400 nm; and the ratio of the average outer micropore diameter ( $D_o$ ) to the average inner micropore diameter ( $D_i$ ) is at least 1.5:1 and the following equation holds:

$$0.3 \leq P_o \leq 0.6;$$

and

the hydrophilic layer comprises a polymer comprising recurring units derived from acrylic acid, and the hydrophilic layer is present at a dry coverage of at least 0.005 g/m<sup>2</sup> and up to and including 0.08 g/m<sup>2</sup>.

This invention also provides a method for providing a lithographic printing plate, comprising:

imagewise exposing the lithographic printing plate precursor of any embodiment of the present invention to imaging radiation to form an imagewise exposed imageable layer having exposed regions and non-exposed regions, and

removing either the exposed regions or the non-exposed regions, but not both exposed regions and non-exposed regions, from the imagewise exposed imageable layer, to form a lithographic printing plate.

In addition, the present invention provides a method for preparing a lithographic printing plate precursor, comprising, in order:

providing an aluminum-containing plate having an electrochemically or mechanically grained and etched planar surface;

subjecting the aluminum-containing plate to a first anodizing process to form an outer aluminum oxide layer on the electrochemically or mechanically grained and etched planar surface, the outer aluminum oxide layer: comprising a multiplicity of outer micropores having an average outer micropore diameter ( $D_o$ ) of at least 15 nm and up to and including 30 nm; having an average dry thickness ( $T_o$ ) of at least 130 nm and up to and including 650 nm; and having a micropore density of at least 500 pores/ $\mu\text{m}^2$  and up to and including 3,000 micropores/ $\mu\text{m}^2$ ; wherein the average outer micropore diameter ( $D_o$ ) in nanometers and the micropore density ( $C_o$ ) in micropores/ $\mu\text{m}^2$ , are further constrained by the porosity ( $P_o$ ) of the outer aluminum oxide layer according to the following equation:

25

$$0.3 \leq P_o \leq 0.8$$

wherein  $P_o$  is defined as  $3.14(C_o)(D_o)^2/4,000,000$ ;

rinsing the outer aluminum oxide layer;

subjecting the aluminum-containing plate to a second anodizing process to form an inner aluminum oxide layer underneath the outer aluminum oxide layer, the inner aluminum oxide layer having: an average dry thickness ( $T_i$ ) of at least 650 nm and up to and including 3,000 nm; and comprising a multiplicity of inner micropores having an

35 average inner micropore diameter ( $D_i$ ) of less than or equal to 15 nm, wherein the ratio of the average outer micropore diameter ( $D_o$ ) to the average inner micropore diameter ( $D_i$ ) is greater than 1.1:1;

rinsing the outer aluminum oxide layer and the inner aluminum oxide layer;

forming a radiation-sensitive imageable layer on the outer aluminum oxide layer; and

optionally, before forming the radiation-sensitive imageable layer on the outer aluminum oxide layer, providing a hydrophilic layer comprising one or more hydrophilic polymers on the outer aluminum oxide layer at a dry coverage of at least 0.0002 g/m<sup>2</sup> and up to and including 0.1 g/m<sup>2</sup>.

The combination of features defined for the substrate used in the lithographic printing plate precursors of the present invention provides improved scratch resistance while maintaining desired on-press developability and high press life. These advantages are achieved by using a unique combination of two anodizing processes that are carried out in such a manner as to achieve the recited features of both the inner and outer aluminum oxide layers that form the inventive substrates in the precursors. As the data provided herein demonstrate, when either or both aluminum oxide layers are outside the required limits, one or more of scratch resistance, on-press developability, and press life are reduced or impaired in some manner.

#### BRIEF DESCRIPTION OF THE DRAWING

FIG. 1 is a black-and-white, cross-sectional scanning electron micrograph (SEM) image of an inventive substrate prepared according to the present invention and having an outer aluminum oxide layer having an average dry thickness

( $T_o$ ) of 218 nm and an inner aluminum oxide layer having an average dry thickness ( $T_i$ ) of 1040 nm.

#### DETAILED DESCRIPTION OF THE INVENTION

The following discussion is directed to various embodiments of the present invention and while some embodiments can be desirable for specific uses, the disclosed embodiments should not be interpreted or otherwise considered to limit the scope of the present invention, as claimed below. In addition, one skilled in the art will understand that the following disclosure has broader application than is explicitly described and the discussion of any embodiment.

#### Definitions

As used herein to define various components of the radiation-sensitive imageable layer formulations (and resulting dried layers), processing solutions, anodizing solutions, hydrophilic layer formulations (and resulting dried layers), and other materials used in the practice of this invention, unless otherwise indicated, the singular forms "a," "an," and "the" are intended to include one or more of the components (that is, including plurality referents).

Each term that is not explicitly defined in the present application is to be understood to have a meaning that is commonly accepted by those skilled in the art. If the construction of a term would render it meaningless or essentially meaningless in its context, the term should be interpreted as having a standard dictionary meaning.

The use of numerical values in the various ranges specified herein, unless otherwise expressly indicated otherwise, are considered to be approximations as though the minimum and maximum values within the stated ranges were both preceded by the word "about." In this manner, slight variations above and below the stated ranges may be useful to achieve substantially the same results as the values within the ranges. In addition, the disclosure of these ranges is intended as a continuous range including every value between the minimum and maximum values as well as the end points of the ranges.

Unless the context indicates otherwise, when used herein, the terms "negative-working radiation-sensitive lithographic printing plate precursor," "positive-working radiation-sensitive lithographic printing plate," "precursor," "radiation-sensitive precursor," and "lithographic printing plate precursor" are meant to be equivalent references of certain embodiments of the present invention.

The term "support" is used herein to refer to an aluminum-containing or other metal-containing material (sheet, web, strip, sheet, foil, or other form) that can be then treated to prepare a "substrate" as described in more detail below.

Average outer micropore diameter ( $D_o$ ) in nanometers (nm) can be determined from a top view SEM image at a magnification of at least 50,000 $\times$  taken from the substrate surface before the application of the optional hydrophilic layer and the radiation-sensitive imageable layer or layers. It is also possible to determine the outer micropore diameter ( $D_o$ ) of a lithographic printing plate precursor by striping the organic layers with appropriate solvents and optionally removing about 20 nm to 80 nm thick outer portion of the outer aluminum oxide layer using an appropriate technique such as argon ion beam sputtering before taking the top view of the SEM image. The average can be determined by reviewing over 200 outer micropores.

Average inner micropore diameter ( $D_i$ ) can be determined from a cross-sectional view SEM image at a magnification of at least 50,000 $\times$ . The cross-section can be generated by bending the lithographic printing plate precursor or its substrate after the imageable layers and the optional hydrophilic layer have been removed. During bending, cracks are formed in the aluminum oxide layer and new surfaces are formed usually at the weakest position, which is usually located at the thinnest walls between adjacent inner micropores. Therefore, the new surfaces of cracks provide cross-sectional views of many micropores. For the present invention, it is not necessary to determine the exact average inner micropore diameter ( $D_i$ ) as long as at least 90% of revealed micropore cross-sections has a width below 15 nm.

Average dry thickness ( $T_o$ ) of the outer anodizing layer and average dry thickness ( $T_i$ ) of the inner anodizing layer, in nanometers (nm), each can be determined from the cross-section SEM images of at least 50,000 $\times$  magnification. The cross-sections of the aluminum oxide layer can be revealed through the cracks formed by bending a lithographic printing plate precursor or its substrate. The cross-sections of the aluminum oxide layer can also be revealed by cutting a slot through the aluminum oxide layer by a focused ion beam (FIB), a technique well known in the art.

The outer anodizing layer micropore density ( $C_o$ ), in micropores/ $\mu\text{m}^2$ , can be determined from the top view SEM pictures of at least 50,000 $\times$  magnification by counting the number of micropores in a predetermined area of a square having an area of at least 500 nm by 500 nm.

The porosity ( $P_o$ ) of the outer aluminum oxide layer can be constrained by either of the following equations:

$$0.3 \leq P_o \leq 0.8 \text{ or}$$

$$0.3 \leq P_o \leq 0.6,$$

wherein  $P_o$  is defined as  $3.14(C_o)(D_o)^2/4,000,000$ .

As used herein, the term "radiation absorber" refers to a compound or material that absorbs electromagnetic radiation in a defined region and typically refers to compounds or materials that have an absorption maximum in the region of at least 250 nm (UV and violet) and up to and including 1400 nm.

As used herein, the term "infrared region" refers to radiation having a wavelength of at least 750 nm and higher. In most instances, the term "infrared" is used to refer to the "near-infrared" region of the electromagnetic spectrum that is defined herein to be at least 750 nm and up to and including 1400 nm. Similarly, infrared radiation absorbers provide sensitivity in the infrared region.

For clarification of definitions for any terms relating to polymers, reference should be made to "Glossary of Basic Terms in Polymer Science" as published by the International Union of Pure and Applied Chemistry ("IUPAC"), *Pure Appl. Chem.* 68, 2287-2311 (1996). However, any definitions explicitly set forth herein should be regarded as controlling.

As used herein, the term "polymer" is used to describe compounds with relatively large molecular weights formed by linking together many small reacted monomers. As the polymer chain grows, it folds back on itself in a random fashion to form coiled structures. With the choice of solvents, a polymer can become insoluble as the chain length grows and become polymeric particles dispersed in the solvent medium. These particle dispersions can be very stable and useful in radiation-sensitive imageable layers described for use in the present invention. In this invention, unless indicated otherwise, the term "polymer" refers to a

non-crosslinked material. Thus, crosslinked polymeric particles differ from the non-crosslinked polymeric particles in that the latter can be dissolved in certain organic solvents of good solvating property whereas the crosslinked polymeric particles may swell but do not dissolve in the organic solvent because the polymer chains are connected by strong covalent bonds.

The term "copolymer" refers to polymers composed of two or more different repeating or recurring units that are arranged along the copolymer backbone.

The term "polymer backbone" refers to the chain of atoms in a polymer to which a plurality of pendant groups can be attached. An example of such a polymer backbone is an "all carbon" backbone obtained from the polymerization of one or more ethylenically unsaturated polymerizable monomers. Some polymer backbones can comprise both carbon and heteroatoms if the polymer is formed using condensation polymerization reactions using suitable reactants.

Recurring units in polymeric binders described herein are generally derived from the corresponding ethylenically unsaturated polymerizable monomers used in a polymerization process, which ethylenically unsaturated polymerizable monomers can be obtained from various commercial sources or prepared using known chemical synthetic methods.

As used herein, the term "ethylenically unsaturated polymerizable monomer" refers to a compound comprising one or more ethylenically unsaturated ( $-C=C-$ ) bonds that are polymerizable using free radical or acid-catalyzed polymerization reactions and conditions. It is not meant to refer to chemical compounds that have only unsaturated  $-C=C-$  bonds that are not polymerizable under these conditions.

Unless otherwise indicated, the term "weight %" refers to the amount of a component or material based on the total solids of a composition, formulation, or dry layer. Unless otherwise indicated, the percentages can be the same for either a dry layer or the total solids of the formulation or composition used to form that dry layer.

As used herein, the term "layer" or "coating" can consist of one disposed or applied layer or a combination of several sequentially disposed or applied layers. If a layer is considered radiation-sensitive and negative-working, it is both sensitive to suitable radiation (for example infrared radiation) and negative-working in the formation of lithographic printing plates. Similarly, if a layer is considered radiation-sensitive and positive-working, it is both sensitive to infrared radiation and positive-working in the formation of lithographic printing plates.

#### Uses

The lithographic printing plate precursors of the present invention are useful for forming lithographic printing plates for lithographic printing using a lithographic printing ink and fountain solution. These precursors are prepared with the structure and components described as follows. In addition, the present invention is useful for preparing such lithographic printing plates by imagewise exposing and processing the exposed precursor off-press using a suitable developer or on-press using a lithographic printing ink, a fountain solution, or a combination of a lithographic printing ink and a fountain solution as described below. The lithographic printing plate precursors of the present invention can be designed to be either negative-working or positive-working using the appropriate materials and manufacturing procedures described below.

The present invention is also useful for manufacturing of such lithographic printing plate precursors that can then be sold to customers for use in imaging and printing.

#### Inventive Substrate

The inventive substrates useful in the present invention are designed with critical features and properties in order to achieve the advantages described above.

A general description relating to the production of substrates useful for lithographic printing plate precursors can be found in US Patent Application Publication 2014/0047993 A1 (noted above) the disclosure of which is herein incorporated by reference for details not explicitly provided herein.

In general, the lithographic printing plate substrate can be derived from an aluminum or other metal material, such as an aluminum alloy containing up to 10% by weight of one or more elements including but not limited to, manganese, silicon, iron, titanium, copper, magnesium, chromium, zinc, bismuth, nickel, and zirconium. The aluminum- or aluminum alloy-containing support (or "plate" or "raw stock") can have any form from which it can be further processed, including sheets, continuous webs and coiled strips as long as it has at least one planar surface that can be treated as described below to form a hydrophilic planar surface in the inventive substrates. It is also possible to use polymeric films or papers onto which pure aluminum- or aluminum alloy-containing layers are deposited or laminated.

The resulting substrate should be thick enough to mechanically withstand the conditions in a modern printing press, but thin enough to be installed on (or wrapped around) a printing cylinder of such a machine. Thus, the substrates should also have appropriate tensile strength, elasticity, crystallinity, and conductivity needed for lithographic printing. These properties can be achieved by standard methods such as heat treatments or cold and hot rolling typical for the fabrication of continuous lithographic support strips, webs, or coils. Dry thicknesses of the resulting inventive substrates are generally at least 100  $\mu\text{m}$  and up to and including 600  $\mu\text{m}$ .

The described aluminum-containing supports can be treated using typical lithographic printing plate precursor manufacturing processes, including pre-etch, water rinse, roughening, water rinse, post-etch, and final water rinse, in combination with the first and second anodizing process described in more detail below.

The raw stock aluminum-containing support is typically subjected to a pre-etching step to remove oil, grease, and metallic or other contaminants at or near the planar surface. As is known in the art, this pre-etching step can be carried using a sodium hydroxide or other aqueous alkaline solutions or even certain organic solvents at known concentrations, times, and temperatures. A separate or additional degreasing step can be carried out using an aqueous surfactant solution if desired. A skilled worker would be able to carry out routine experimentation to find the optimal pre-etching conditions (for example, optimal solution concentration, dwell time, and temperature).

Typically, after the pre-etching step, the etched support is "roughened" in a suitable manner such as by using a known electrochemical or mechanical roughening (or graining) process. In electrochemical graining treatments, the etched support can be processed with alternating electric current in a solution of 5 to 20 g/liter hydrochloric acid. It is also possible to use solutions of nitric acid (for example, at up to 2.5 weight %) or sulfuric acid or mixtures for this purpose. Such electrochemical graining solutions can also contain additives such as corrosion inhibitors and stabilizers, including but not limited to metal nitrates, metal chlorides, monoamines, diamines, aldehydes, phosphoric acid, chromic acid, boric acid, lactic acid, acetic acid, and oxalic acid. For

example, electrochemical graining can be carried out using the processes described in U.S. Patent Application Publication 2008/0003411 (Hunter et al.), the disclosure of which is incorporated herein by reference. A skilled worker would be able to determine by routine experimentation the optimal conditions for either electrochemical or mechanical graining as such processes are well known in the art. Mechanical graining processes can be carried out for example with suitable brushes alone or in combination with a slurry of abrasive materials such as silica particles or alumina particles. Alternatively, a combination of mechanical and electrochemical graining processes can be used.

During roughening or graining, smut can be formed on the planar surface of the support and this smut can be removed in a post-etching step using a treatment with a highly acidic or highly alkaline solution, for example, to remove 0.01-5.0 g/m<sup>2</sup> of the support surface. For example, post-etching can be carried out using a solution of sodium hydroxide, trisodium phosphate, or sulfuric acid. The amount of post-etching can be controlled by setting dwell time, concentration, and temperature of the etching solution. A suitable amount of post-etching also depends on the amount of roughening and the amount of smut formed in that step. The post-etching treatment must be sufficient to remove the smut, but it should not destroy too much of the surface structures formed in the roughening step. The post-etching treatment must be sufficient to remove the smut, but it should not destroy too much of the surface structures formed in the roughening step. Thus, there are many combinations of the parameters that a skilled artisan can consider during routine experimentation to find the optimum post-etching conditions.

The foregoing steps result in an electrochemically or mechanically grained (roughened) and etched planar surface in the aluminum-containing support.

The next steps carried out according to the present invention include a first anodizing process and a second anodizing process, both of which are essential to the present invention, to form outer and inner aluminum oxide layers, respectively. The method of the present invention does not require additional anodizing processes (that is, third or more anodizing processes) as are sometimes described in the prior art, so that in most embodiments, the first and second anodizing processes described herein are the only anodizing processes. If a third anodizing process is carried out, it can be achieved with relatively high voltage but low charge density in order to enhance the barrier layer between the inner micropores and the aluminum-containing support, and the dry thickness of the resulting third (innermost) aluminum oxide layer is less than 5% of the thickness of the inner aluminum oxide layer formed during the second anodizing process.

The first and second anodizing processes can be generally carried out using sulfuric or phosphoric acid (electrolyte) solutions at a suitable time of at least 20° C. and up to and including 70° C. for at least 1 second and up to and including 250 seconds, sufficient to provide a total dry aluminum oxide coverage (total for both outer and inner aluminum oxide layers) of up to and including 4 g/m<sup>2</sup>. The conditions are described as follows for both the first and second anodizing processes.

A suitable aluminum-containing plate having an electrochemically or mechanically grained and etched planar surface is subjected to a first anodizing process to form an outer aluminum oxide layer on that electrochemically or mechanically grained and etched planar surface. The first anodizing process can be carried out, for example, using an electrolyte composition containing at least 50 g/liter and up to and

including 350 g/liter of phosphoric acid or at least 150 g/liter and up to and including 300 g/liter of sulfuric acid, and a suitable amount of aluminum, for example 5 g/liter. These solution amounts can be optimized as to type of acid, acid concentration, aluminum concentration, dwell time, and temperature in order to achieve the desired outer aluminum oxide layer properties as described herein. Representative details of such first anodizing process are illustrated in the working Examples described below. It is particularly useful to carry out the first anodizing process using phosphoric acid.

The resulting outer aluminum oxide layer should comprise a multiplicity of outer micropores having an average outer micropore diameter ( $D_o$ ) of at least 15 nm and up to and including 30 nm. In addition, the average dry thickness ( $T_o$ ) of the outer aluminum oxide layer is at least 130 nm and up to and including 650 nm, or is more likely at least 130 nm and up to and including 400 nm. The micropore density ( $C_o$ ) of the outer anodizing layer is generally at least 500 micropores/ $\mu\text{m}^2$  and up to and including 3,000 micropores/ $\mu\text{m}^2$ .

Moreover, the average outer micropore diameter ( $D_o$ ) in nanometers and the micropore density ( $C_o$ ) in micropores/ $\mu\text{m}^2$  of the outer aluminum oxide layer are further constrained or related according to either of the following equations:

$$0.3 \leq P_o \leq 0.8 \text{ or}$$

$$0.3 \leq P_o \leq 0.6,$$

wherein  $P_o$  is defined above.

Once the first anodizing process has been carried out for the desired time, the formed outer aluminum oxide layer can be rinsed, if desired, with a suitable solution such as water at a suitable temperature and time to remove residual acid and aluminum, and to stop the first anodizing process.

Unlike some processes known in the art, such as U.S. Patent Application Publication 2013/0052582 (Hayashi), the method of the present invention does not include what is known in the art as a “pore widening” (or micropore widening) step following anodization. Thus, such treatments are not purposely used in the practice of the present invention.

The second anodizing process is then carried out to form an inner aluminum oxide layer underneath the outer aluminum oxide layer, using a suitable electrolyte composition that can comprise at least 100 g/liter and up to and including 350 g/liter of sulfuric acid as well as a suitable amount of aluminum, for example 5 g/liter. These solution amounts can be optimized as to acid concentration, aluminum concentration, dwell time, and temperature in order to achieve the desired inner aluminum oxide layer properties as described herein. The details of such second anodizing process are illustrated in the working Examples described below.

The resulting inner aluminum oxide layer disposed on the grained and etched planar surface of the substrate should comprise a multiplicity of inner micropores having an average inner micropore diameter ( $D_i$ ) of less than or equal to 15 nm and typically less than or equal to 10 nm. In addition, the average dry thickness ( $T_i$ ) of the inner aluminum oxide layer is at least 650 nm or at least 700 nm, and up to and including 1500 nm, or up to and including 3,000 nm.

In addition, it is highly important that the ratio of the average outer micropore diameter ( $D_o$ ) be greater than the average inner micropore diameter ( $D_i$ ), for example, the

## 11

ratio of  $D_o$  to  $D_i$  is greater than 1.1:1, or even greater than 1.5:1, and typically, greater than 2:1.

Once the second anodizing process is carried out for a desired time, both formed outer aluminum oxide layer and inner aluminum oxide layer can be rinsed, if desired, with a suitable solution such as water, at a suitable temperature and time to remove residual acid and aluminum, and to stop the second anodizing process.

While it is not essential, it is usually desirable to provide a hydrophilic layer on the outer aluminum oxide layer in what is sometimes known in the art as a “post-treatment”. When used, the hydrophilic layer can be provided from a hydrophilic layer formulation comprising one or more hydrophilic polymers to provide a dry coverage of the hydrophilic layer of at least 0.0002 g/m<sup>2</sup> and up to and including 0.1 g/m<sup>2</sup> or in an amount of at least 0.005 g/m<sup>2</sup> and up to and including 0.08 g/m<sup>2</sup>. Useful hydrophilic polymers include but are not limited to, homopolymers and copolymers derived at least in part from any of acrylic acid, acrylic acid, methacrylamide, acrylamide, vinyl phosphoric acid dimethyl ester, and vinyl phosphonic acid, and combinations thereof. Particularly useful hydrophilic polymers comprise recurring units derived from either acrylic acid or methacrylic acid, or both. Useful hydrophilic polymers can be purchased from a number of commercial sources or prepared using known ethylenically unsaturated polymerizable monomers and polymerization reaction conditions. The hydrophilic layer and the hydrophilic layer formulation can contain additives such as inorganic acid (for example, phosphoric acid in an amount of at least 0.01 weight %), salts of inorganic acids, and surfactants. A particularly useful hydrophilic layer formulation is described below in relation to the working Examples.

The post-treatment process can be carried out in any suitable manner as described for examples in [0058]-[0061] of U.S. Patent Application Publication 2014/0047993 (note above). Alternatively, the post-treatment process can be carried out by coating a desired amount of the hydrophilic layer formulation in a suitable solvent such as water directly onto the outer aluminum oxide layer and then drying the resulting wet coating.

After all of these essential and optional treatments, the resulting inventive substrates, in any suitable form such as flat sheets or continuous webs or coils, are ready for the preparation of lithographic printing plate precursors according to the present invention.

## Radiation-Sensitive Imageable Layers and Precursors

One or more radiation-sensitive imageable layers can be formed on the outer aluminum oxide layer (or on the hydrophilic layer if present) in a suitable manner using suitable radiation-sensitive imageable layer formulations as described in more detail below. Such radiation-sensitive imageable layers can be positive-working or negative-working in chemical nature.

## Negative-Working Lithographic Printing Plate Precursors:

In some embodiments, the precursors of the present invention can be formed by suitable application of a negative-working radiation-sensitive composition as described below to a suitable substrate (as described above) to form a radiation-sensitive imageable layer that is negative-working on that substrate. In general, the radiation-sensitive composition (and resulting radiation-sensitive imageable layer) comprises (a) one or more free radically polymerizable components, (b) an initiator composition that provides free radicals upon exposure to imaging radiation, and (c) one or more radiation absorbers, as essential components, and

## 12

optionally, a polymeric binder different from all of (a), (b), and (c), all of which essential and optional components are described in more detail below. There is generally only a single radiation-sensitive imageable layer in the precursor. It is generally the outermost layer in the precursor, but in some embodiments, there can be an outermost water-soluble hydrophilic overcoat (also known as a topcoat or oxygen bather layer) disposed over the radiation-sensitive imageable layer.

It is particularly useful to design the components of the radiation-sensitive imageable layer in such a manner (types and forms of chemical compounds and amounts of each) that after imagewise exposure, it is on-press developable using a lithographic printing ink, a fountain solution, or a combination of a lithographic printing ink and a fountain solution. More details of on-press developability are described below.

The radiation-sensitive composition (and radiation-sensitive imageable layer prepared therefrom) comprises (a) one or more free radically polymerizable components, each of which contains one or more free radically polymerizable groups (and two or more of such groups in some embodiments) that can be polymerized using free radical initiation. In some embodiments, the radiation-sensitive imageable layer comprises two or more free radically polymerizable components having the same or different numbers of free radically polymerizable groups in each molecule.

Useful free radically polymerizable components can contain one or more free radical polymerizable monomers or oligomers having one or more addition polymerizable ethylenically unsaturated groups (for example, two or more of such groups). Similarly, crosslinkable polymers having such free radically polymerizable groups can also be used. Oligomers or prepolymers, such as urethane acrylates and methacrylates, epoxide acrylates and methacrylates, polyester acrylates and methacrylates, polyether acrylates and methacrylates, and unsaturated polyester resins can be used. In some embodiments, the free radically polymerizable component comprises carboxyl groups.

It is possible for one or more free radically polymerizable components to have large enough molecular weight to enhance the mechanical properties of the radiation-sensitive imageable layer and thus make the corresponding lithographic printing plate precursors suitable for transportation in typical packaging and for handling during normal pre-press operation. It is also possible for one or more free radically polymerizable components to be present in the radiation-sensitive layer as a particulate material, the components having a particle size of at least 10 nm and up to and including 800 nm. In such embodiments, a separate non-polymerizable or non-crosslinkable polymer binder (described below) is not necessary but may still be present.

Free radically polymerizable components include urea urethane (meth)acrylates or urethane (meth)acrylates having multiple (two or more) polymerizable groups. Mixtures of such compounds can be used, each compound having two or more unsaturated polymerizable groups, and some of the compounds having three, four, or more unsaturated polymerizable groups. For example, a free radically polymerizable component can be prepared by reacting DESMODUR® N100 aliphatic polyisocyanate resin based on hexamethylene diisocyanate (Bayer Corp., Milford, Conn.) with hydroxyethyl acrylate and pentaerythritol triacrylate. Useful free radically polymerizable compounds include NK Ester A-DPH (dipentaerythritol hexaacrylate) that is available from Kowa American, and Sartomer 399 (dipentaerythritol pentaacrylate), Sartomer 355 (di-trimethylolpropane tetraacrylate), Sartomer 295 (pentaerythritol tetraacrylate), and

Sartomer 415 [ethoxylated (20)trimethylolpropane triacrylate] that are available from Sartomer Company, Inc.

Numerous other free radically polymerizable components are known in the art and are described in considerable literature including *Photoreactive Polymers: The Science and Technology of Resists*, A Reiser, Wiley, New York, 1989, pp. 102-177, by B. M. Monroe in *Radiation Curing: Science and Technology*, S. P. Pappas, Ed., Plenum, New York, 1992, pp. 399-440, and in "Polymer Imaging" by A. B. Cohen and P. Walker, in *Imaging Processes and Material*, J. M. Sturge et al. (Eds.), Van Nostrand Reinhold, New York, 1989, pp. 226-262. For example, useful free radically polymerizable components are also described in EP 1,182,033A1 (Fujimaki et al.), beginning with paragraph [0170], and in U.S. Pat. No. 6,309,792 (Hauck et al.), U.S. Pat. No. 6,569,603 (Furukawa), and U.S. Pat. No. 6,893,797 (Munnelly et al.) the disclosures of all of which are incorporated herein by reference. Other useful free radically polymerizable components include those described in U.S. Patent Application Publication 2009/0142695 (Baumann et al.), which radically polymerizable components include 1H-tetrazole groups, the disclosure of which is incorporated herein by reference.

Useful free radically polymerizable components as described above can be readily obtained from various commercial sources or prepared using known starting materials and synthetic methods.

The (a) one or more free radically polymerizable components are generally present in a radiation-sensitive imageable layer in an amount of at least 10 weight % and up to and including 70 weight %, or typically of at least 20 weight % and up to and including 50 weight %, all based on the total dry weight of the radiation-sensitive imageable layer.

The radiation-sensitive imageable layer used in the present invention also comprises includes (b) an initiator composition that provides free radicals in the presence of a suitable radiation absorber, upon exposure of the radiation-sensitive imageable layer to suitable imaging radiation to initiate the polymerization of the one or more free radically polymerizable components. The initiator composition can be a single compound or a combination or system of a plurality of compounds.

Suitable initiator compositions include but are not limited to, aromatic sulfonylhalides; trihalogenoalkylsulfones; trihalogenoarylsulfones; imides (such as N-benzoyloxyphthalimide); diazosulfonates; 9,10-dihydroanthracene derivatives; N-aryl, S-aryl, or O-aryl polycarboxylic acids with at least 2 carboxy groups, of which at least one is bonded to the nitrogen, oxygen, or sulfur atom of the aryl moiety; oxime esters and oxime ethers;  $\alpha$ -hydroxy- or  $\alpha$ -amino-acetophenones; benzoin ethers and esters; peroxides; hydroperoxides; azo compounds; 2,4,5-triarylimidazoyl dimers (such as "HABI's"); trihalomethyl substituted triazines; boron-containing compounds; organoborate salts such as those described in U.S. Pat. No. 6,562,543 (Ogata et al.), and onium salts.

Useful initiator compositions particularly for infrared radiation-sensitive compositions and imageable layers include but are not limited to, onium salts such as ammonium, iodonium, sulfonium, and phosphonium compounds that are described in detail in [0131] of U.S. Patent Application Publication 2014/0047993 (noted above), and references cited therein, the disclosures of which are incorporated herein by reference. Examples of the onium salts include triphenylsulfonium, diphenyliodonium, diphenyldiazonium, and derivatives obtained by introducing one or more substituents into the benzene ring of these compounds. Suitable

substituents include but are not limited to, alkyl, alkoxy, alkoxy carbonyl, acyl, acyloxy, chloro, bromo, fluoro and nitro groups.

Examples of anions in the onium salts include but are not limited to, halogen anions,  $\text{ClO}_4^-$ ,  $\text{PF}_6^-$ ,  $\text{BF}_4^-$ ,  $\text{SbF}_6^-$ ,  $\text{CH}_3\text{SO}_3^-$ ,  $\text{CF}_3\text{SO}_3^-$ ,  $\text{C}_6\text{H}_5\text{SO}_3^-$ ,  $\text{CH}_3\text{C}_6\text{H}_4\text{SO}_3^-$ ,  $\text{HOC}_6\text{H}_4\text{SO}_3^-$ ,  $\text{CIC}_6\text{H}_4\text{SO}_3^-$ , and boron anion as described for example in U.S. Pat. No. 7,524,614 (Tao et al.), the disclosure of which is incorporated herein by reference.

The onium salt can be obtained by combining an onium salt having sulfonium in the molecule with an onium salt in the molecule. The onium salt can be a polyvalent onium salt having at least two onium ion atoms in the molecule that are bonded through a covalent bond. Among polyvalent onium salts, those having at least two onium ion atoms in the molecule are useful and those having a sulfonium or iodonium cation in the molecule are particularly useful. Representative polyvalent onium salts are represented by the following formulas (6) and (7):

(6)



(7)



Furthermore, the onium salts described in paragraphs [0033] to of the specification of Japanese Patent Publication 2002-082429 [or U.S. Patent Application Publication 2002-0051934 (Ippei et al.), the disclosure of which is incorporated herein by reference] or the iodonium borate complexes described in U.S. Pat. No. 7,524,614 (noted above), can also be used in the present invention.

In some embodiments, the initiator composition can comprise a combination of initiator compounds such as a combination of iodonium salts, for example the combination of Compound A and Compound B described as follows.

Compound A can be represented by Structure (I) shown below, and the one or more compounds collectively known as compound B can be represented below by either Structure (II) or (III):

(I)

 $\text{X}_1^-$

15

-continued



In these Structures (I), (II), and (III), R<sub>1</sub>, R<sub>2</sub>, R<sub>3</sub>, R<sub>4</sub>, R<sub>5</sub> and R<sub>6</sub> are independently substituted or unsubstituted alkyl groups or substituted or unsubstituted alkoxy groups, each of these alkyl or alkoxy groups having from 2 to 9 carbon atoms (or particularly from 3 to 6 carbon atoms). These substituted or unsubstituted alkyl and alkoxy groups can be in linear or branched form. In many useful embodiments, R<sub>1</sub>, R<sub>2</sub>, R<sub>3</sub>, R<sub>4</sub>, R<sub>5</sub> and R<sub>6</sub> are independently substituted or unsubstituted alkyl groups, such as independently chosen substituted or unsubstituted alkyl groups having 3 to 6 carbon atoms.

In addition, at least one of R<sub>3</sub> and R<sub>4</sub> can be different from R<sub>1</sub> or R<sub>2</sub>; the difference between the total number of carbon atoms in R<sub>1</sub> and R<sub>2</sub> and the total number of carbon atoms in R<sub>3</sub> and R<sub>4</sub> is 0 to 4 (that is, 0, 1, 2, 3, or 4); the difference between the total number (sum) of carbon atoms in R<sub>1</sub> and R<sub>2</sub> and the total number (sum) of carbon atoms in R<sub>5</sub> and R<sub>6</sub> is 0 to 4 (that is, 0, 1, 2, 3, or 4); and X<sub>1</sub>, X<sub>2</sub> and X<sub>3</sub> are the same or different anions.

Useful anions include but are not limited to, ClO<sub>4</sub><sup>-</sup>, PF<sub>6</sub><sup>-</sup>, BF<sub>4</sub><sup>-</sup>, SbF<sub>6</sub><sup>-</sup>, CH<sub>3</sub>SO<sub>3</sub><sup>-</sup>, CF<sub>3</sub>SO<sub>3</sub><sup>-</sup>, C<sub>6</sub>H<sub>5</sub>SO<sub>3</sub><sup>-</sup>, CH<sub>3</sub>C<sub>6</sub>H<sub>4</sub>SO<sub>3</sub><sup>-</sup>, HOC<sub>6</sub>H<sub>4</sub>SO<sub>3</sub><sup>-</sup>, ClC<sub>6</sub>H<sub>4</sub>SO<sub>3</sub><sup>-</sup>, and borate anions represented by the following Structure (IV):



wherein R<sup>1</sup>, R<sup>2</sup>, R<sup>3</sup>, and R<sup>4</sup> independently represent substituted or unsubstituted alkyl, substituted or unsubstituted aryl (including halogen-substituted aryl groups), substituted or unsubstituted alkenyl, substituted or unsubstituted alkynyl, substituted or unsubstituted cycloalkyl, or substituted or unsubstituted heterocyclic groups, or two or more of R<sup>1</sup>, R<sup>2</sup>, R<sup>3</sup>, and R<sup>4</sup> can be joined together to form a substituted or unsubstituted heterocyclic ring with the boron atom, such rings having up to 7 carbon, nitrogen, oxygen, or nitrogen atoms. The optional substituents on R<sup>1</sup>, R<sup>2</sup>, R<sup>3</sup>, and R<sup>4</sup> can include chloro, fluoro, nitro, alkyl, alkoxy, and acetoxy groups. In some embodiments, all of the R<sup>1</sup>, R<sup>2</sup>, R<sup>3</sup>, and R<sup>4</sup> are the same or different substituted or unsubstituted aryl groups such as substituted or unsubstituted phenyl groups, or more likely all of these groups are unsubstituted phenyl groups. In many embodiments, at least one of X<sub>1</sub>, X<sub>2</sub>, and X<sub>3</sub> is a tetraarylborate anion comprising the same or different aryl groups, or in particularly useful embodiments, one or more is a tetraphenylborate anion or each of X<sub>1</sub>, X<sub>2</sub>, and X<sub>3</sub> is a tetraphenylborate anion.

Mixtures of Compound B compounds represented by Structures (II) or (III) can be used if desired. Many useful compounds represented by Structures (I), (II), and (III) can

16

be obtained from commercial sources such as Sigma-Aldrich or they can be prepared using known synthetic methods and readily available starting materials.

Components useful in the initiator compositions described above can be obtained from various commercial sources or prepared using known synthetic methods and starting materials.

The initiator composition is generally present in the radiation-sensitive imageable layer sufficient to provide one or more polymerization initiators in an amount of at least 0.5 weight % and up to and including 20 weight %, or typically of at least 2 weight % and up to and including 15 weight %, or even of at least 4 weight % and up to and including 12 weight %, all based on the total dry weight of the radiation-sensitive imageable layer.

In addition, the radiation-sensitive imageable layer also comprises (c) one or more radiation absorbers to provide desired radiation sensitivity or to convert radiation to heat, or both. In some embodiments, the radiation-sensitive layer is sensitive to infrared radiation and comprises one or more different infrared radiation absorbers so that the lithographic printing plate precursors can be imaged with infrared radiation-emitting lasers. The present invention is also applicable to lithographic printing plate precursors designed for imaging with violet lasers having emission peaks at around 405 nm, with visible lasers such as those having emission peaks around 488 nm or 532 nm, or with UV radiation having significant emission peaks below 400 nm. In such embodiments, the radiation absorbers can be selected to match the radiation source and many useful examples are known in the art, and are sometimes called "sensitizers". Useful radiation absorbers of this types are described for example, in Col. 11 (lines 10-43) of U.S. Pat. No. 7,285,372 (Baumann et al.), the disclosure of which is incorporated herein by reference.

In most embodiments of the present invention, the radiation-sensitive imageable layer comprises one or more infrared radiation absorbers to provide desired infrared radiation sensitivity. Useful infrared radiation absorbers can be pigments or infrared radiation absorbing dyes. Suitable dyes also can be those described in for example, U.S. Pat. No. 5,208,135 (Patel et al.), U.S. Pat. No. 6,153,356 (Urano et al.), U.S. Pat. No. 6,309,792 (Hauck et al.), U.S. Pat. No. 6,569,603 (Furukawa), U.S. Pat. No. 6,797,449 (Nakamura et al.), U.S. Pat. No. 7,018,775 (Tao), U.S. Pat. No. 7,368,45 (Munnelly et al.), U.S. Pat. No. 8,632,941 (Balbinot et al.), and U.S. Patent Application Publication 2007/056457 (Iwai et al.), the disclosures of all of which are incorporated herein by reference. In some infrared radiation-sensitive embodiments, it is desirable that at least one infrared radiation absorber in the infrared radiation-sensitive imageable layer be a cyanine dye comprising a tetraarylborate anion such as a tetraphenylborate anion. Examples of such dyes include those described in United States Patent Application Publication 2011/003123 (Simpson et al.) the disclosure of which is incorporated herein by reference.

In addition to low molecular weight IR-absorbing dyes, IR dye chromophores bonded to polymers can be used as well. Moreover, IR dye cations can be used as well, that is, the cation is the IR absorbing portion of the dye salt that ionically interacts with a polymer comprising carboxy, sulfo, phospho, or phosphono groups in the side chains.

Useful radiation absorbers described above can be readily obtained from various commercial sources or prepared using known starting materials and synthetic methods.

The total amount of one or more radiation absorbers in the radiation-sensitive imageable layer is at least 0.5 weight % and up to and including 30 weight %, or typically of at least

1 weight % and up to and including 15 weight %, based on the total dry weight of the radiation-sensitive imageable layer.

It is optional but desirable in many embodiments that the radiation-sensitive imageable layer further comprise one or more (d) polymeric binders (or materials that act as polymeric binders) for all of the materials in the noted layer. Such polymer binders are different from all of the (a), (b), and (c) materials described above. These polymeric binders are generally non-crosslinkable and non-polymerizable.

Such (d) polymeric binders can be selected from a number of polymeric binder materials known in the art including polymers comprising recurring units having side chains comprising polyalkylene oxide segments such as those described in for example, U.S. Pat. No. 6,899,994 (Huang et al.) the disclosure of which is incorporated herein by reference. Other useful (d) polymeric binders comprise two or more types of recurring units having different side chains comprising polyalkylene oxide segments as described in for example WO Publication 2015-156065 (Kamiya et al.). Some of such (d) polymeric binders can further comprise recurring units having pendant cyano groups as those described in for example U.S. Pat. No. 7,261,998 (Hayashi et al.) the disclosure of which is incorporated herein by reference.

Some useful (d) polymeric binders can be present in particulate form, that is, in the form of discrete, non-agglomerated particles. Such discrete particles can have an average particle size of at least 10 nm and up to and including 1500 nm, or typically of at least 80 nm and up to and including 600 nm, and are generally distributed uniformly within the radiation-sensitive imageable layer. For example, one or more useful (d) polymeric binders can be present in the form of particles having an average particle size of at least 50 nm and up to and including 400 nm. Average particle size can be determined by various known methods including measuring the particles in electron scanning microscope images, and averaging a set number of measurements.

In some embodiments, the (d) polymeric binder is present in the form of particles having an average particle size that is less than the average dry thickness (t) of the radiation-sensitive imageable layer. The average dry thickness (t) in micrometers ( $\mu\text{m}$ ) is calculated by the following Equation:

$$t=w/r$$

wherein w is the dry coating coverage of the radiation-sensitive imageable layer in  $\text{g}/\text{m}^2$  and r is  $1\text{ g}/\text{cm}^3$ . For example, in such embodiments, the (d) polymeric binder can comprise at least 0.05% and up to and including 80%, or more likely at least 10% and up to and including 50%, of the radiation-sensitive imageable layer.

The (d) polymeric binders also can have a backbone comprising multiple (at least two) urethane moieties as well as pendant groups comprising the polyalkylenes oxide segments.

Other useful (d) polymeric binders can comprise polymerizable groups such as acrylate ester, methacrylate ester, vinyl aryl, and allyl groups and as well as alkali soluble groups such as carboxylic acid. Some of these useful (d) polymeric binders are described in U.S. Patent Application Publication 2015/0099229 (Simpson et al.) and U.S. Pat. No. 6,916,595 (Fujimaki et al.), the disclosures of both of which are incorporated herein by reference.

Useful (d) polymeric binders generally have a weight average molecular weight ( $M_w$ ) of at least 2,000 and up to and including 500,000, or at least 20,000 and up to and

including 300,000, as determined by Gel Permeation Chromatography (polystyrene standard).

Useful (d) polymeric binders can be obtained from various commercial sources or they can be prepared using known procedures and starting materials, as described for example in publications described above.

The total (d) polymeric binders can be present in the radiation-sensitive imageable layer in an amount of at least 10 weight % and up to and including 70 weight %, or more likely in an amount of at least 20 weight % and up to and including 50 weight %, based on the total dry weight of the radiation-sensitive imageable layer.

Other polymeric materials known in the art (different from the (d) polymeric binders) can be present in the radiation-sensitive imageable layer and such polymeric materials are generally more hydrophilic or more hydrophobic than the (d) polymeric binders described above. Example of such hydrophilic polymeric binders include but are not limited to, cellulose derivatives such as hydroxypropyl cellulose, carboxymethyl cellulose, and polyvinyl alcohol with various degrees of saponification. More hydrophobic polymeric binders are less developable than the (d) polymeric binders described above and typically have an acid value less than 20 mg KOH/g for all acidic groups having a pKa below 7 and their corresponding salts. Such hydrophobic polymeric binders typically contain less than 10 weight %, more typically less than 5 weight %, segments that contribute to the hydrophilicity of the binder and are selected from the group consisting of hydroxyl group,  $-\text{CH}_2\text{CH}_2-\text{O}-$  and  $-\text{C}(=\text{O})\text{NH}_2$ . Examples of such hydrophobic polymeric binders include but are not limited to, poly(methyl methacrylate), poly(benzyl methacrylate), and polystyrene.

Additional optional additives to the radiation-sensitive imageable layer can include organic dyes or organic dye precursors and color developers as are known in the art. Useful organic dyes or organic dye precursors include but are not limited to, phthalide and fluoran leuco dyes having a lactone skeleton with an acid dissociable lactone skeleton, such as those described in U.S. Pat. No. 6,858,374 (Yanaka), the disclosure of which is incorporated herein by reference. Such optional additives can be used as print-out colorants and can be present in an amount of at least 1 weight % and up to and including 10 weight %, based on the total dry weight of the radiation-sensitive imageable layer. Other useful print-out colorants are known in the art and can include azo dyes, triarylmethane dyes, cyanine dyes, and spirolactone or spirolactam colorants as described for example in U.S. Patent Application Publication 2009/0047599 (Horne et al.).

The radiation-sensitive imageable layer can include cross-linked polymer particles having an average particle size of at least 2  $\mu\text{m}$ , or of at least 4  $\mu\text{m}$ , and up to and including 20  $\mu\text{m}$  as described for example in U.S. Pat. No. 8,383,319 (Huang et al.), U.S. Pat. No. 8,105,751 (Endo et al.), and U.S. Pat. No. 9,366,962 (Kamiya et al.), the disclosures of all of which are incorporated herein by reference. Such cross-linked polymeric particles can be present only in the radiation-sensitive imageable layer, only in the hydrophilic overcoat when present (described below), or in both the radiation-sensitive imageable layer and the hydrophilic overcoat when present.

The radiation-sensitive imageable layer can also include a variety of other optional addenda including but not limited to, dispersing agents, humectants, biocides, plasticizers, surfactants for coatability or other properties, viscosity builders, pH adjusters, drying agents, defoamers, preserva-

tives, antioxidants, development aids, rheology modifiers, or combinations thereof, or any other addenda commonly used in the lithographic art, in conventional amounts. The radiation-sensitive imageable layer can also include a phosphate (meth)acrylate having a molecular weight generally greater than 250 as described in U.S. Pat. No. 7,429,445 (Munnely et al.) the disclosure of which is incorporated herein by reference.

#### Hydrophilic Overcoat:

While in some embodiments of the negative-working lithographic printing plate precursors, the radiation-sensitive imageable layer is the outermost layer with no layers disposed thereon, it is possible that the precursors can be designed with a hydrophilic layer (also known in the art as a hydrophilic overcoat, oxygen-barrier layer, or topcoat) disposed directly on the radiation-sensitive imageable layer (no intermediate layers between these two layers). Such precursors can be developed on-press as well as off-press using any suitable developer as described below. When present, this hydrophilic overcoat is generally the outermost layer of the precursor.

Such hydrophilic overcoats can comprise one or more film-forming water-soluble polymeric binders in an amount of at least 60 weight % and up to and including 100 weight %, based on the total dry weight of the hydrophilic overcoat. Such film-forming water-soluble (or hydrophilic) polymeric binders can include a modified or unmodified poly(vinyl alcohol) having a saponification degree of at least 30%, or a degree of at least 75%, or a degree of at least 90%, and a degree of up to and including 99.9%.

Further, one or more acid-modified poly(vinyl alcohol) can be used as film-forming water-soluble (or hydrophilic) polymeric binders in the hydrophilic overcoat. For example, at least one modified poly(vinyl alcohol) can be modified with an acid group selected from the group consisting of carboxylic acid, sulfonic acid, sulfuric acid ester, phosphonic acid, and phosphoric acid ester groups. Examples of such materials include but are not limited to, sulfonic acid-modified poly(vinyl alcohol), carboxylic acid-modified poly(vinyl alcohol), and quaternary ammonium salt-modified poly(vinyl alcohol), glycol-modified poly(vinyl alcohol), or combinations thereof.

The hydrophilic overcoat can also include crosslinked polymer particles having an average particle size of at least 2  $\mu\text{m}$  and as described for example in U.S. Pat. No. 8,383,319 (Huang et al.) and U.S. Pat. No. 8,105,751 (Endo et al.), the disclosures of both of which are incorporated herein by reference.

The hydrophilic overcoat can be provided at a dry coating coverage of at least 0.1  $\text{g}/\text{m}^2$  and up to but less than 4  $\text{g}/\text{m}^2$ , and typically at a dry coating coverage of at least 0.15  $\text{g}/\text{m}^2$  and up to and including 2.5  $\text{g}/\text{m}^2$ . In some embodiments, the dry coating coverage is as low as 0.1  $\text{g}/\text{m}^2$  and up to and including 1.5  $\text{g}/\text{m}^2$  or at least 0.1  $\text{g}/\text{m}^2$  and up to and including 0.9  $\text{g}/\text{m}^2$ , such that the hydrophilic overcoat is relatively thin.

The hydrophilic overcoat can optionally comprise organic wax particles dispersed within the one or more film-forming water-soluble (or hydrophilic) polymeric binders as described for example in U.S. Patent Application Publication 2013/0323643 (Balbinot et al.) the disclosure of which is incorporated herein by reference.

#### Positive-Working Lithographic Printing Plate Precursors:

Some embodiments of the present invention are precursors that are positive-working and comprise one or more radiation-sensitive imageable layers disposed on the inventive substrate described above. Some of such precursors

comprise a single radiation-sensitive imageable layer disposed on the substrate, while other precursors are two-layer ("dual-layer") precursors comprising at least an inner radiation-sensitive imageable layer disposed on the substrate and an outer radiation-sensitive imageable layer disposed over the inner radiation-sensitive imageable layer.

The positive-working lithographic printing plate precursors of the present invention are designed for imaging using infrared radiation and therefore contain one or more infrared radiation absorbers (like those described above) dispersed in one or more alkali-soluble polymers that, upon suitable infrared irradiation, are soluble, dispersible, or removable in an alkaline solution (that is, an alkaline developer) such as used for processing (development) of such exposed precursors. Thus, the one or more positive-working radiation-sensitive imageable layers undergo a change in solubility properties with respect to the processing solution in their irradiated (exposed) regions. The one or more infrared radiation absorbers can be present in one or more of the layers present in the precursor.

For the two-layer or "dual-layer" positive-working lithographic printing plate precursors, the inner layer (also known as the under layer) is disposed on the inventive substrate, and the outer layer (also known as the top layer) is generally disposed over the inner layer. An intermediate layer between the inner and outer radiation-sensitive layers can be present if desired. Before thermal imaging, the outer layer is generally not soluble or removable by an alkaline developer with the usual time allotted for development, but after thermal imaging, the exposed regions of the outer layer are soluble in the alkaline developer. The inner layer is also generally removable by an alkaline developer.

Materials (both essential and optional materials) that are useful in both "single-layer" and "dual-layer" lithographic printing plate precursors, structures of such precursors, and methods of making such precursors, are known in the art. Many details are provided in [0067]-[0111] of U.S. Patent Application Publication 2014/0047993 (noted above), the disclosure of which is incorporated herein by reference.

#### Making Lithographic Printing Plate Precursors

The radiation-sensitive lithographic printing plate precursors of the present invention can be provided in the following manner. A radiation-sensitive imageable layer formulation comprising materials described above (for either negative-working or positive-working chemistry) can be applied to the inventive substrate, usually in a continuous substrate roll or web, as described above using any suitable equipment and procedure, such as spin coating, knife coating, gravure coating, die coating, slot coating, bar coating, wire rod coating, roller coating, or extrusion hopper coating. The radiation-sensitive imageable layer formulation can also be applied by spraying onto a suitable substrate. Typically, once the radiation-sensitive imageable layer formulation is applied at a suitable wet coverage, it is dried in a suitable manner known in the art to provide a desired dry coverage as noted below, thereby providing a radiation-sensitive continuous article that can be in any suitable form such as a web from which individual precursors can be prepared using known manufacturing processes.

For the dual-layer positive-working lithographic printing plate precursors, once an inner radiation-sensitive layer formulation has been applied to the inventive substrate, an outer radiation-sensitive layer formulation can then be applied, usually in a sequential continuous manufacturing operation, followed by drying both inner and outer radia-

tion-sensitive imageable layers. Intermixing of the two imageable layer formulations should be avoided as much as possible.

The manufacturing methods typically include mixing the various components needed for a particular radiation-sensitive imageable layer chemistry in a suitable organic solvent or mixtures thereof [such as methyl ethyl ketone (2-butanone), methanol, ethanol, 1-methoxy-2-propanol, iso-propyl alcohol, acetone,  $\gamma$ -butyrolactone, n-propanol, tetrahydrofuran, and others readily known in the art, as well as mixtures thereof], applying the resulting infrared radiation-sensitive imageable layer formulation to the continuous substrate web, and removing the solvent(s) by evaporation under suitable drying conditions. The selection of organic solvents (or mixtures thereof) can be chosen for dual-layer positive-working lithographic printing plate precursors so that the two layer formulations are not mixed to a significant extent and the inner layer formulation is not dissolved when the outer layer formulation is applied. Further details of such manufacturing features are described in U.S. Patent Application Publication 2014/0047993 (noted above).

After proper drying, the dry coverage of the negative-working radiation-sensitive imageable layer (especially those that are infrared radiation-sensitive) on an inventive substrate is generally at least 0.1 g/m<sup>2</sup> and up to and including 4 g/m<sup>2</sup> or at least 0.4 g/m<sup>2</sup> and up to and including 2 g/m<sup>2</sup> but other dry coverage amounts can be used if desired.

For single-layer positive-working lithographic printing plate precursors, the dry coverage of the single radiation-sensitive imageable layer is generally at least 0.5 g/m<sup>2</sup> and up to and including 2.5 g/m<sup>2</sup> or at least 1 g/m<sup>2</sup> and up to and including 2 g/m<sup>2</sup>.

For dual-layer positive-working lithographic printing plate precursors, the dry coverage for the inner radiation-sensitive imageable layer is generally at least 0.2 g/m<sup>2</sup> and up to and including 2.5 g/m<sup>2</sup> or at least 0.5 g/m<sup>2</sup> and up to and including 2 g/m<sup>2</sup>; and the dry coverage for the outer radiation-sensitive imageable layer is generally at least 0.2 g/m<sup>2</sup> and up to and including 2 g/m<sup>2</sup> or at least 0.3 g/m<sup>2</sup> and up to and including 1 g/m<sup>2</sup>.

As described above, in some negative-working precursor embodiments, a suitable aqueous-based hydrophilic overcoat formulation can be applied to the dried radiation-sensitive imageable layer using known coating and drying conditions, equipment, and procedures.

In practical manufacturing conditions, the result of these coating operations is a continuous web or roll of radiation-sensitive lithographic printing plate precursor material having either one or more radiation-sensitive imageable layers and any optional layers noted above disposed on the inventive substrate described above.

Individual rectangular lithographic printing plate precursors are formed from this resulting continuous radiation-sensitive web or roll by slitting to create multiple longitudinal strips, each of which has a width equal to one dimension of rectangular lithographic printing plate precursors. A cutting-to-length process is used to create a lateral cut across each strip at an interval equal to the other dimension of rectangular lithographic printing plate precursors, thereby forming individual precursors having a square or rectangular form.

#### Imaging (Exposing) Conditions

During use, a radiation-sensitive lithographic printing plate precursor of this invention can be exposed to a suitable source of exposing radiation depending upon the radiation absorber (or sensitizer) present in the one or more radiation-

sensitive imageable layers. For example, most of the negative-working and all of the positive-working lithographic printing plate precursors can be imaged with infrared lasers that emit significant radiation within the range of at least 750 nm and up to and including 1400 nm, or of at least 800 nm and up to and including 1250 nm. However, some negative-working lithographic printing plate precursors can be imaged in the UV, "violet," or visible regions of the electromagnetic spectrum using suitable sources of imaging radiation (for example, from 250 nm and less than 750 nm). The result of such imagewise exposure is to provide exposed regions and non-exposed regions in the one or more radiation-sensitive imageable layers.

15 Imaging can be carried out using imaging or exposing radiation from a radiation-generating laser (or array of such lasers). Imaging also can be carried out using imaging radiation at multiple wavelengths at the same time if desired, for example, using multiple infrared radiation wavelengths. 20 The laser used to expose the precursor is usually a diode laser, because of the reliability and low maintenance of diode laser systems, but other lasers such as gas or solid-state lasers can also be used. The combination of power, intensity and exposure time for radiation imaging would be 25 readily apparent to one skilled in the art.

The imaging apparatus can be configured as a flatbed recorder or as a drum recorder, with the radiation-sensitive lithographic printing plate precursor mounted to the interior or exterior cylindrical surface of the drum. An example of 30 useful infrared imaging apparatus is available as models of KODAK® Trendsetter platesetters (Eastman Kodak Company) and NEC AMZISetter X-series (NEC Corporation, Japan) that contain laser diodes that emit radiation at a wavelength of about 830 nm. Other suitable infrared imaging apparatus includes the Screen PlateRite 4300 series or 35 8600 series platesetters (available from Screen USA, Chicago, Ill.) or thermal CTP platesetters from Panasonic Corporation (Japan) that operate at a wavelength of 810 nm.

Infrared radiation imaging energies can be at least 30 40 mJ/cm<sup>2</sup> and up to and including 500 mJ/cm<sup>2</sup> and typically at least 50 mJ/cm<sup>2</sup> and up to and including 300 mJ/cm<sup>2</sup> depending upon the sensitivity of the infrared radiation-sensitive imageable layer.

Useful UV and "violet" imaging apparatus include Pro- 45 setter (Heidelberger Druckmaschinen, Germany), Luxel V8/V6 series (Fuji, Japan), Python (Highwater, UK), MakoNews, Mako 2, and Mako 8 (ECRM, US), Micro (Screen, Japan), Polaris and Advantage (AGFA, Belgium), LS Jet (Multiformat) and Smart 'n' Easy Jet (Krause, 50 Germany), and VMAX series (DotLine, Germany), imag-setters.

55 Imaging in the UV to visible region of the electromagnetic spectrum and particularly the UV region (250 nm to 450 nm) can be carried out using energies of at least 0.01 mJ/cm<sup>2</sup> and up to and including 0.5 mJ/cm<sup>2</sup> at a power density of at least 0.5 kW/cm<sup>2</sup> and up to and including 50 kW/cm<sup>2</sup>.

#### Processing (Development) and Printing

##### Exposed Positive-Working Precursors:

These precursors are typically processed after exposure 60 off-press using a suitable developer and apparatus that are known in the art, for a time sufficient to remove the exposed regions of the one or more exposed radiation-sensitive imageable layers to reveal the hydrophilic outer surface of the inventive substrate prepared according to the present invention, and leaving intact the non-exposed regions. Suitable developers, apparatus, conditions for processing, and 65 any optional pre- or post-development treatments use would

be readily apparent to one skilled in the art and some details of this type are described in [0150]-[0152].

Printing using the imagewise exposed and processed positive-working lithographic printing plate precursors can be carried out using known printing presses, lithographic printing inks, fountain solutions, and printing conditions. Some details of printing processed are provided below in relation to the exposed and processed lithographic printing plates. Lithographic printing ink would be preferentially attracted to the remaining non-exposed regions on the lithographic printing surface of resulting lithographic printing plates and repelled by the hydrophilic surface of the inventive substrate in the exposed regions.

Exposed Negative-Working Precursors:

After imagewise exposing, the exposed negative-working radiation-sensitive lithographic printing plate precursors having exposed regions and non-exposed regions in the radiation-sensitive imageable layer can be processed in a suitable manner to remove the non-exposed regions and any hydrophilic overcoat if present, and leaving intact the hardened exposed regions.

Processing can be carried out off-press using any suitable developer in one or more successive applications (treatments or developing steps) of the same or different processing solution (developer). Such one or more successive processing treatments can be carried out for a time sufficient to remove the non-exposed regions of the radiation-sensitive imageable layer to reveal the outermost hydrophilic surface of the inventive substrate, but not long enough to remove significant amounts of the exposed regions that have been hardened in the same layer. During lithographic printing, the revealed hydrophilic surface of the inventive substrate repels ink while the remaining exposed regions accept lithographic printing ink.

Prior to such off-press processing, the exposed precursors can be subjected to a "pre-heating" process to further harden the exposed regions in the radiation-sensitive imageable layer. Such optional pre-heating can be carried out using any known process and equipment generally at a temperature of at least 60° C. and up to and including 180° C.

Following this optional pre-heating, or in place of the pre-heating, the exposed precursor can be washed (rinsed) to remove any hydrophilic overcoat that is present. Such optional washing (or rinsing) can be carried out using any suitable aqueous solution (such as water or an aqueous solution of a surfactant) at a suitable temperature and for a suitable time that would be readily apparent to one skilled in the art.

Useful developers can be ordinary water or formulated aqueous solutions. The formulated developers can comprise one or more components selected from surfactants, organic solvents, alkali agents, and surface protective agents. For example, useful organic solvents include the reaction products of phenol with ethylene oxide and propylene oxide [such as ethylene glycol phenyl ether (phenoxyethanol)], benzyl alcohol, esters of ethylene glycol and of propylene glycol with acids having 6 or less carbon atoms, and ethers of ethylene glycol, diethylene glycol, and of propylene glycol with alkyl groups having 6 or less carbon atoms, such as 2-ethylethanol and 2-butoxyethanol.

In some instances, an aqueous processing solution can be used off-press to both develop the imaged precursor by removing the non-exposed regions and also to provide a protective layer or coating over the entire imaged and developed (processed) precursor printing surface. In this embodiment, the aqueous solution behaves somewhat like a gum that is capable of protecting (or "gumming") the

lithographic image on the printing plate against contamination or damage (for example, from oxidation, fingerprints, dust, or scratches).

After the described off-press processing and optional drying, the resulting lithographic printing plate can be mounted onto a printing press without any contact with additional solutions or liquids. It is optional to further bake the lithographic printing plate with or without blanket or flood-wise exposure to UV or visible radiation.

10 Printing can be carried out by applying a lithographic printing ink and fountain solution to the printing surface of the lithographic printing plate in a suitable manner. The fountain solution is taken up by the hydrophilic surface of the inventive substrate revealed by the exposing and processing steps, and the lithographic ink is taken up by the remaining (exposed) regions of the radiation-sensitive imageable layer. The lithographic ink is then transferred to a suitable receiving material (such as cloth, paper, metal, glass, or plastic) to provide a desired impression of the 15 image thereon. If desired, an intermediate "blanket" roller 20 can be used to transfer the lithographic ink from the lithographic printing plate to the receiving material (for example, sheets of paper).

On-Press Development and Printing:

25 Alternatively, the negative-working lithographic printing plate precursors of the present invention are on-press developable using a lithographic printing ink, a fountain solution, or a combination of a lithographic printing ink and a fountain solution. In such embodiments, an imaged radiation-sensitive lithographic printing plate precursor according to the present invention is mounted onto a printing press and the printing operation is begun. The non-exposed regions in the radiation-sensitive imageable layer are removed by a suitable fountain solution, lithographic printing ink, or a combination of both, when the initial printed 30 impressions are made. Typical ingredients of aqueous fountain solutions include pH buffers, desensitizing agents, surfactants and wetting agents, humectants, low boiling solvents, biocides, antifoaming agents, and sequestering agents. A representative example of a fountain solution is 35 Varn Litho Etch 142W+Yarn PAR (alcohol sub) (available from Varn International, Addison, Ill.).

In a typical printing press startup with a sheet-fed printing machine, the dampening roller is engaged first and supplies 40 fountain solution to the mounted imaged precursor to swell the exposed radiation-sensitive imageable layer at least in the non-exposed regions. After a few revolutions, the inking rollers are engaged and they supply lithographic printing ink(s) to cover the entire printing surface of the lithographic 45 printing plates. Typically, within 5 to 20 revolutions after the inking roller engagement, printing sheets are supplied to remove the non-exposed regions of the radiation-sensitive imageable layer from the lithographic printing plate as well as materials on a blanket cylinder if present, using the 50 formed ink-fountain solution emulsion.

On-press developability of infrared radiation exposed lithographic printing precursors is particularly useful when the precursor comprises one or more polymeric binders in an infrared radiation-sensitive imageable layer, at least one of 55 which polymeric binders is present as particles having an average diameter of at least 50 nm and up to and including 400 nm.

The present invention provides at least the following 60 embodiments and combinations thereof, but other combinations of features are considered to be within the present invention as a skilled artisan would appreciate from the teaching of this disclosure:

1. A lithographic printing plate precursor comprising:  
a substrate having a planar surface, and  
a radiation-sensitive imageable layer disposed over the planar surface of the substrate, or in some embodiments, one or more radiation-sensitive imageable layers disposed over the planar surface of the substrate (such as in positive-working lithographic printing plate precursors),

wherein the substrate comprises:

an aluminum-containing plate having a grained and etched planar surface;

an inner aluminum oxide layer disposed on the grained and etched planar surface, the inner aluminum oxide layer having an average dry thickness ( $T_i$ ) of at least 650 nm and up to and including 3,000 nm; and comprising a multiplicity of inner micropores having an average inner micropore diameter ( $D_i$ ) of less than or equal to 15 nm;

an outer aluminum oxide layer disposed on the inner aluminum oxide layer, the outer aluminum oxide layer comprising a multiplicity of outer micropores having an average outer micropore diameter ( $D_o$ ) of at least 15 nm and up to and including 30 nm; having an average dry thickness ( $T_o$ ) of at least 130 nm and up to and including 650 nm; and having a micropore density ( $C_o$ ) of at least 500 micropores/ $\mu\text{m}^2$  and up to and including 3,000 micropores/ $\mu\text{m}^2$ , wherein the ratio of the average outer micropore diameter ( $D_o$ ) to the average inner micropore diameter ( $D_i$ ) is greater than 1.1:1, and the average outer micropore diameter ( $D_o$ ) in nanometers and the micropore density ( $C_o$ ) in micropores/ $\mu\text{m}^2$ , are further constrained by the porosity ( $P_o$ ) of the outer aluminum oxide layer according to the following equation:

$$0.3 \leq P_o \leq 0.8$$

wherein  $P_o$  is defined as  $3.14(C_o)(D_o^2)/4,000,000$ ; and

optionally a hydrophilic layer comprising one or more hydrophilic polymers, which hydrophilic layer is disposed on the outer aluminum oxide layer at a dry coverage of at least 0.0002 g/m<sup>2</sup> and up to and including 0.1 g/m<sup>2</sup>.

2. A method for preparing the lithographic printing plate precursor of embodiment 1, comprising, in order:

providing an aluminum-containing plate having an electrochemically or mechanically grained and etched planar surface;

subjecting the aluminum-containing plate to a first anodizing process to form an outer aluminum oxide layer on the electrochemically or mechanically grained and etched planar surface, the outer aluminum oxide layer comprising a multiplicity of outer micropores having an average outer micropore diameter ( $D_o$ ) of at least 15 nm and up to and including 30 nm; having an average dry thickness ( $T_o$ ) of at least 130 nm and up to and including 650 nm; and having a micropore density of at least 500 pores/ $\mu\text{m}^2$  and up to and including 3,000 micropores/ $\mu\text{m}^2$ ; wherein the average outer micropore diameter ( $D_o$ ) in nanometers and the micropore density ( $C_o$ ) in micropores/ $\mu\text{m}^2$ , are further constrained by the porosity ( $P_o$ ) of the outer aluminum oxide layer according to the following equation:

$$0.3 \leq P_o \leq 0.8$$

wherein  $P_o$  is defined as  $3.14(C_o)(D_o^2)/4,000,000$ ;

rinsing the outer aluminum oxide layer;

subjecting the aluminum-containing plate to a second anodizing process to form an inner aluminum oxide layer underneath the outer aluminum oxide layer, the inner aluminum oxide layer having an average dry thickness ( $T_i$ ) of at least 650 nm and up to and including 3,000 nm; and comprising a multiplicity of inner micropores having an average inner micropore diameter ( $D_i$ ) of less than or equal

to 15 nm, wherein the ratio of the average outer micropore diameter ( $D_o$ ) to the average inner micropore diameter ( $D_i$ ) is greater than 1.1:1;

rinsing the outer aluminum oxide layer and the inner aluminum oxide layer;

forming a radiation-sensitive imageable layer on the outer aluminum oxide layer (or forming one or more radiation-sensitive imageable layers on the outer aluminum oxide layer as in the case of manufacturing positive-working lithographic printing plate precursors); and

optionally, before forming the radiation-sensitive imageable layer on the outer aluminum oxide layer, providing a hydrophilic layer comprising one or more hydrophilic polymers on the outer aluminum oxide layer at a dry coverage of at least 0.0002 g/m<sup>2</sup> and up to and including 0.1 g/m<sup>2</sup>.

3. The method of embodiment 2, wherein the first anodizing process is carried out using phosphoric acid.

4. Any of embodiments 1 to 3, wherein the outer aluminum oxide layer has an average dry thickness ( $T_o$ ) of at least 150 nm and up to and including 400 nm.

5. Any of embodiments 1 to 4, wherein the inner aluminum oxide layer has an average dry thickness ( $T_i$ ) of at least 700 nm and up to and including 1500 nm.

6. Any of embodiments 1 to 5, wherein the following equation holds:

$$0.3 \leq P_o \leq 0.6.$$

7. Any of embodiments 1 to 6, wherein the ratio of the average outer micropore diameter ( $D_o$ ) to the average inner micropore diameter ( $D_i$ ) is at least 1.5:1.

8. Any of embodiments 1 to 7, further comprising the hydrophilic layer that comprises one or more water-soluble polymers, at least one of which water-soluble polymers comprises recurring units derived from either acrylic acid or methacrylic acid, or both acrylic acid and methacrylic acid.

9. Any of embodiments 1 to 8, wherein the radiation-sensitive imageable layer is sensitive to infrared radiation and comprises one or more infrared radiation absorbers.

10. Any of embodiments 1 to 9, wherein the radiation-sensitive imageable layer is positive-working and comprises one or more alkali-soluble polymers that are removable from the substrate upon exposure to radiation.

11. Any of embodiments 1 to 9, wherein the radiation-sensitive imageable layer is negative-working and comprises:

(a) one or more free radically polymerizable components;  
(b) an initiator composition that provides free radicals upon exposure of the radiation-sensitive imageable layer to radiation;  
(c) one or more radiation absorbers; and optionally,  
(d) a polymeric binder that is different from all of (a), (b), and (c).

12. Embodiment 11, wherein the radiation-sensitive imageable layer is infrared radiation-sensitive and the one or more radiation absorbers comprise one or more infrared radiation absorbers.

13. Any of embodiments 1 to 9, 11, and 12, wherein the radiation-sensitive layer is negative-working and is on-press developable.

14. Any of embodiments 1 to 9 and 11 to 13, wherein the radiation-sensitive layer further comprises the (d) polymeric binder that is in particulate form.

15. Any of embodiments 1, 4 to 9, 13, and 14, wherein the lithographic printing plate precursor is negative-working and further comprises a hydrophilic overcoat disposed over the radiation-sensitive imageable layer.

16. Any of embodiments 1 to 9 and 11 to 15, wherein: the grained and etched planar surface of the aluminum-containing plate has been electrochemically grained and etched;

the radiation-sensitive imageable layer is a negative-working and on-press developable infrared radiation-sensitive imageable layer that is disposed on the electrochemically grained and etched planar surface, and comprises:

- (a) one or more free radically polymerizable components;
  - (b) an initiator composition that provides free radicals upon exposure of the radiation-sensitive imageable layer to infrared radiation;
  - (c) one or more infrared radiation absorbers; and
  - (d) a particulate polymeric binder that is different from all of (a), (b), and (c);

the inner aluminum oxide layer has an average dry thickness ( $T_i$ ) of at least 700 nm and up to and including 1,500 nm;

the outer aluminum oxide layer has an average dry thickness ( $T_o$ ) of at least 130 nm and up to and including 400 nm; and the ratio of the average outer micropore diameter ( $D_o$ ) to the average inner micropore diameter ( $D_i$ ) is at least 1.5:1 and the following equation holds:

$$0.3 \leq P_o \leq 0.6;$$

and

the hydrophilic layer comprises a polymer comprising recurring units derived from acrylic acid, and the hydrophilic layer is present at a dry coverage of at least 0.005 g/m<sup>2</sup> and up to and including 0.08 g/m<sup>2</sup>.

17. A method for providing a lithographic printing plate, comprising:

imagewise exposing the lithographic printing plate precursor of any of embodiments 1 and 4-16 to imaging radiation to form an imagewise exposed imageable layer having exposed regions and non-exposed regions, and

removing either the exposed regions or the non-exposed regions, but not both exposed regions and non-exposed regions, from the imagewise exposed imageable layer, to form a lithographic printing plate.

18. The method of embodiment 17, wherein the non-exposed regions in the imagewise exposed imageable layer are removed.

19. The method of embodiment 18, wherein the non-exposed regions in the imagewise exposed imageable layer are removed on-press using a lithographic printing ink, a fountain solution, or both the lithographic printing ink and the fountain solution.

20. The method of any of embodiments 17 to 19, wherein the imagewise exposing is carried out using infrared radiation.

10 The following Examples are provided to illustrate the practice of this invention and are not meant to be limiting in any manner.

## Invention Examples 1-31

Inventive aluminum-containing substrates used in Invention Examples 1-31 were prepared according to the general processes described above. Hydro 1052 aluminum alloy strip or web (available from Norsk Hydro ASA, Norway) having a thickness of 0.28 mm was used as the aluminum-containing "plate" stock or support. Both pre-etch and post-etch steps were carried out in alkaline solutions under known conditions. Roughening (or graining) was carried out by electrochemical means in a hydrochloric acid solution at about 23° C. to obtain an arithmetic average roughness (Ra) of 0.5  $\mu$ m on a planar surface of the aluminum-containing support. These treatment steps were carried out in a continuous process on a typical manufacturing line used to manufacture lithographic printing plate precursors. The resulting grained and etched aluminum-containing support was then rinsed with water, dried, and cut into individual grained and etched aluminum-containing sheets. Each individual sheet was then anodized twice wherein each anodizing process bath contained about 100 liters of anodizing solution. The first and second anodizing conditions for each of the Invention Examples 1-31 are shown below in TABLE I. The first anodizing process to form the outer aluminum oxide layer was carried out using phosphoric acid as the electrolyte and the second anodizing process to form the inner aluminum oxide layer was carried out using sulfuric acid as the electrolyte.

TABLE I

| Conditions for First and Second Anodizing Processes |                             |                    |                                      |            |                                     |                             |                    |                                      |            |                                     |
|-----------------------------------------------------|-----------------------------|--------------------|--------------------------------------|------------|-------------------------------------|-----------------------------|--------------------|--------------------------------------|------------|-------------------------------------|
| Invention Example                                   | First Anodizing Treatment   |                    |                                      |            |                                     | Second Anodizing Treatment  |                    |                                      |            |                                     |
|                                                     | Electrolyte conc. [g/liter] | Temperature [° C.] | Current density [A/dm <sup>2</sup> ] | Time [sec] | Charge density [C/dm <sup>2</sup> ] | Electrolyte conc. [g/liter] | Temperature [° C.] | Current density [A/dm <sup>2</sup> ] | Time [sec] | Charge density [C/dm <sup>2</sup> ] |
| 1                                                   | 175                         | 60                 | 4.7                                  | 15.0       | 70.7                                | 280                         | 23                 | 10.0                                 | 18.0       | 180.0                               |
| 2                                                   | 150                         | 60                 | 3.8                                  | 32.6       | 123.7                               | 280                         | 23                 | 10.0                                 | 18.0       | 180.0                               |
| 3                                                   | 100                         | 60                 | 2.8                                  | 63.1       | 176.7                               | 280                         | 23                 | 10.0                                 | 18.0       | 180.0                               |
| 4                                                   | 200                         | 60                 | 5.5                                  | 46.4       | 255.3                               | 280                         | 23                 | 10.0                                 | 18.0       | 180.0                               |
| 5                                                   | 300                         | 60                 | 8.5                                  | 39.3       | 334.3                               | 280                         | 23                 | 10.0                                 | 18.0       | 180.0                               |
| 6                                                   | 175                         | 60                 | 5.8                                  | 7.6        | 44.2                                | 280                         | 23                 | 10.0                                 | 18.0       | 180.0                               |
| 7                                                   | 175                         | 65                 | 7.8                                  | 9.1        | 70.7                                | 280                         | 23                 | 10.0                                 | 18.0       | 180.0                               |
| 8                                                   | 175                         | 60                 | 5.8                                  | 21.3       | 123.7                               | 280                         | 23                 | 10.0                                 | 18.0       | 180.0                               |
| 9                                                   | 175                         | 55                 | 3.8                                  | 46.5       | 176.7                               | 280                         | 23                 | 10.0                                 | 18.0       | 180.0                               |
| 10                                                  | 175                         | 50                 | 1.8                                  | 120.7      | 217.2                               | 280                         | 23                 | 10.0                                 | 18.0       | 180.0                               |
| 11                                                  | 250                         | 50                 | 9.0                                  | 7.9        | 70.7                                | 280                         | 23                 | 10.0                                 | 18.0       | 180.0                               |
| 12                                                  | 300                         | 50                 | 10.9                                 | 11.4       | 123.7                               | 280                         | 23                 | 10.0                                 | 18.0       | 180.0                               |
| 13                                                  | 200                         | 50                 | 7.1                                  | 25.1       | 176.7                               | 280                         | 23                 | 10.0                                 | 18.0       | 180.0                               |
| 14                                                  | 100                         | 50                 | 3.3                                  | 69.9       | 227.3                               | 280                         | 23                 | 10.0                                 | 18.0       | 180.0                               |
| 15                                                  | 350                         | 55                 | 9.4                                  | 53.7       | 123.4                               | 280                         | 23                 | 10.0                                 | 15.0       | 150.0                               |
| 16                                                  | 350                         | 55                 | 10.5                                 | 13.0       | 44.1                                | 280                         | 23                 | 10.0                                 | 15.0       | 150.0                               |
| 17                                                  | 350                         | 55                 | 14.7                                 | 23.1       | 176.9                               | 280                         | 23                 | 10.0                                 | 15.0       | 150.0                               |
| 18                                                  | 250                         | 55                 | 5.6                                  | 30.7       | 70.7                                | 280                         | 23                 | 10.0                                 | 33.8       | 337.5                               |

TABLE I-continued

| Invention Example | Conditions for First and Second Anodizing Processes |                    |                                      |            |                                     |                             |                    |                                      |            |                                     |
|-------------------|-----------------------------------------------------|--------------------|--------------------------------------|------------|-------------------------------------|-----------------------------|--------------------|--------------------------------------|------------|-------------------------------------|
|                   | First Anodizing Treatment                           |                    |                                      |            | Second Anodizing Treatment          |                             |                    |                                      |            |                                     |
|                   | Electrolyte conc. [g/liter]                         | Temperature [° C.] | Current density [A/dm <sup>2</sup> ] | Time [sec] | Charge density [C/dm <sup>2</sup> ] | Electrolyte conc. [g/liter] | Temperature [° C.] | Current density [A/dm <sup>2</sup> ] | Time [sec] | Charge density [C/dm <sup>2</sup> ] |
| 19                | 250                                                 | 55                 | 6.7                                  | 52.0       | 176.7                               | 280                         | 23                 | 10.0                                 | 33.8       | 337.5                               |
| 20                | 150                                                 | 55                 | 1.8                                  | 53.9       | 123.8                               | 280                         | 23                 | 10.0                                 | 45.0       | 450.0                               |
| 21                | 150                                                 | 55                 | 2.9                                  | 13.1       | 44.7                                | 280                         | 23                 | 10.0                                 | 45.0       | 450.0                               |
| 22                | 150                                                 | 55                 | 7.1                                  | 23.0       | 175.9                               | 280                         | 23                 | 10.0                                 | 45.0       | 450.0                               |
| 23                | 350                                                 | 55                 | 9.4                                  | 53.8       | 123.4                               | 280                         | 23                 | 10.0                                 | 67.5       | 675.0                               |
| 24                | 350                                                 | 55                 | 10.5                                 | 13.1       | 43.6                                | 280                         | 23                 | 10.0                                 | 67.5       | 675.0                               |
| 25                | 350                                                 | 55                 | 14.7                                 | 23.0       | 177.5                               | 280                         | 23                 | 10.0                                 | 67.5       | 675.0                               |
| 28                | 150                                                 | 60                 | 4.6                                  | 48.2       | 219.4                               | 280                         | 23                 | 7.0                                  | 19.3       | 135.0                               |
| 29                | 200                                                 | 55                 | 4.5                                  | 49.3       | 219.4                               | 280                         | 23                 | 10.0                                 | 15.8       | 157.5                               |
| 30                | 250                                                 | 50                 | 4.4                                  | 50.4       | 219.4                               | 280                         | 23                 | 15.0                                 | 10.5       | 157.5                               |
| 31                | 300                                                 | 45                 | 4.3                                  | 51.6       | 219.4                               | 280                         | 23                 | 20.0                                 | 8.0        | 160.0                               |

The micropore structure of each aluminum oxide layer provided by the first and second anodizing processes was evaluated by FE-SEM microscopy, performed on a Hitachi S4100 with a magnification of 50,000 $\times$  to 150,000 $\times$ . Top view SEM micrographs were taken perpendicular to the outer surface of the substrate. Cross-sectional SEM micrographs were taken parallel to the outer surface of the substrate by bending a small sample of each substrate by 180° and inspecting the breaking edge. The dry average layer thickness of each of the inner and outer aluminum oxide layers,  $T_i$  and  $T_o$ , respectively, was measured from several cross-sectional images and the dry average layer thickness is shown below in TABLE II for each Invention Example substrate.

The inner micropore diameters of the inner aluminum oxide layer in the substrate were estimated from the cross-sectional SEM micrographs. The outer micropore diameters of the outer aluminum oxide was determined from the top view SEM micrographs. An average outer micropore diameter ( $D_o$ ) was determined from 200 micropores in three top view SEM micrographs taken at different sample positions and is shown in TABLE II. It was confirmed that the average outer micropore diameter ( $D_o$ ) of the outer aluminum oxide layer at its outer surface was essentially the same as the average outer micropore diameter ( $D_o$ ) below that outer surface. This evaluation was carried out by taking additional

<sup>20</sup> top view SEM micrographs after removing the outermost 50 nm of the outer aluminum oxide layer by a sputtering treatment where the sputter beam ( $Ar^+$  ions) was directed at a sample of the inventive substrate at an angle of 45° relative to the surface normal for a period of time. The sputtering treatment was repeated three times each after rotating the inventive substrate sample by 90° to achieve an even removal across the surface in the SEM viewing area.

<sup>25</sup> FIG. 1 is an SEM image of a representative inventive substrate prepared according to the present invention, having both inner and outer anodizing layers. It is clear that  $T_i$  is much greater than  $T_o$ .

<sup>30</sup> The micropore density ( $C_o$ ) of the outer aluminum oxide layer was determined by counting the micropores per projected surface area of the inventive substrate in the top view SEM micrographs. The porosity of the outer aluminum oxide layer is defined as the area in the top view SEM micrographs covered by micropores relative to the projected surface area parallel to the inventive substrate outermost surface. For micropore diameters smaller than 10 nm, the resolution of the SEM was not high enough to achieve reliable results and thus no information on the inner micropore density and the porosity of the inner aluminum oxide layer is provided.

TABLE II

| Invention Example | Structural Features of the Outer and Inner Aluminum Oxide Layers |                                           |                                             |                        |                                      |                                      |
|-------------------|------------------------------------------------------------------|-------------------------------------------|---------------------------------------------|------------------------|--------------------------------------|--------------------------------------|
|                   | Outer Aluminum Oxide Layer                                       |                                           |                                             |                        | Inner Aluminum Oxide Layer           |                                      |
|                   | Average Dry Thickness ( $T_o$ ) [nm]                             | Average Micropore Diameter ( $D_o$ ) [nm] | Micropore Density [ $1/\mu m^2$ ] ( $C_o$ ) | Porosity (%) ( $P_o$ ) | Average Dry Thickness ( $T_i$ ) [nm] | Average Pore Diameter ( $D_i$ ) [nm] |
| 1                 | 201                                                              | 18                                        | 2709                                        | 67                     | 804                                  | <10                                  |
| 2                 | 304                                                              | 17                                        | 2784                                        | 64                     | 813                                  | <10                                  |
| 3                 | 350                                                              | 18                                        | 2808                                        | 68                     | 817                                  | <10                                  |
| 4                 | 480                                                              | 18                                        | 2667                                        | 65                     | 804                                  | <10                                  |
| 5                 | 595                                                              | 18                                        | 2713                                        | 67                     | 796                                  | <10                                  |
| 6                 | 150                                                              | 19                                        | 1308                                        | 39                     | 809                                  | <10                                  |
| 7                 | 207                                                              | 22                                        | 1292                                        | 48                     | 782                                  | <10                                  |
| 8                 | 340                                                              | 23                                        | 1223                                        | 49                     | 797                                  | <10                                  |
| 9                 | 490                                                              | 23                                        | 1223                                        | 52                     | 803                                  | <10                                  |
| 10                | 580                                                              | 23                                        | 1225                                        | 51                     | 811                                  | <10                                  |
| 11                | 220                                                              | 30                                        | 593                                         | 41                     | 796                                  | <10                                  |
| 12                | 330                                                              | 29                                        | 620                                         | 40                     | 772                                  | <10                                  |

TABLE II-continued

| Structural Features of the Outer and Inner Aluminum Oxide Layers |                                              |                                                   |                                                          |                                |                                              |                                              |
|------------------------------------------------------------------|----------------------------------------------|---------------------------------------------------|----------------------------------------------------------|--------------------------------|----------------------------------------------|----------------------------------------------|
| Invention Example                                                | Outer Aluminum Oxide Layer                   |                                                   |                                                          | Inner Aluminum Oxide Layer     |                                              |                                              |
|                                                                  | Average Dry Thickness (T <sub>o</sub> ) [nm] | Average Micropore Diameter (D <sub>o</sub> ) [nm] | Micropore Density [1/μm <sup>2</sup> ] (C <sub>o</sub> ) | Porosity (%) (P <sub>o</sub> ) | Average Dry Thickness (T <sub>i</sub> ) [nm] | Average Pore Diameter (D <sub>i</sub> ) [nm] |
| 13                                                               | 490                                          | 28                                                | 605                                                      | 37                             | 821                                          | <10                                          |
| 14                                                               | 607                                          | 30                                                | 582                                                      | 41                             | 817                                          | <10                                          |
| 15                                                               | 286                                          | 19                                                | 2780                                                     | 77                             | 663                                          | <10                                          |
| 16                                                               | 155                                          | 20                                                | 1264                                                     | 39                             | 670                                          | <10                                          |
| 17                                                               | 515                                          | 29                                                | 573                                                      | 39                             | 673                                          | <10                                          |
| 18                                                               | 199                                          | 18                                                | 2620                                                     | 63                             | 1499                                         | <10                                          |
| 19                                                               | 481                                          | 22                                                | 1317                                                     | 52                             | 1463                                         | <10                                          |
| 20                                                               | 316                                          | 18                                                | 2799                                                     | 75                             | 1966                                         | <10                                          |
| 21                                                               | 151                                          | 22                                                | 1244                                                     | 48                             | 2019                                         | <10                                          |
| 22                                                               | 510                                          | 28                                                | 601                                                      | 38                             | 2043                                         | <10                                          |
| 23                                                               | 306                                          | 17                                                | 2773                                                     | 61                             | 2944                                         | <10                                          |
| 24                                                               | 165                                          | 20                                                | 1232                                                     | 40                             | 2922                                         | <10                                          |
| 25                                                               | 525                                          | 26                                                | 572                                                      | 30                             | 2966                                         | <10                                          |
| 28                                                               | 619                                          | 21                                                | 1567                                                     | 55                             | 686                                          | <10                                          |
| 29                                                               | 605                                          | 22                                                | 1540                                                     | 60                             | 693                                          | <10                                          |
| 30                                                               | 608                                          | 21                                                | 1473                                                     | 50                             | 697                                          | <10                                          |
| 31                                                               | 608                                          | 19                                                | 1561                                                     | 43                             | 711                                          | <10                                          |

Each of the grained, etched, and anodized substrates thus obtained was further treated (sometimes known as “post-treatment”) to provide a hydrophilic layer over the outer aluminum oxide layer using a hydrophilic layer formulation having the components shown in the following TABLE III, which was applied using a bar coater; dried at 120° C. for 40 seconds; and then cooled to 20-27° C., resulting in a hydrophilic layer dry coverage of 0.03 g/m<sup>2</sup>.

TABLE III

| Hydrophilic Layer Formulation                                                                            |            |
|----------------------------------------------------------------------------------------------------------|------------|
| Component                                                                                                | Amount (g) |
| Polyacrylic acid (PAA) aqueous solution (40 weight %) (obtained as Jurymer AC-10S, marketed by TOAGOSEI) | 3.0        |
| Water                                                                                                    | 27.0       |

Lithographic printing plate precursors were prepared according to the present invention in Invention Examples 1-31 by coating the corresponding inventive substrate described above with a negative-working, radiation-sensitive imageable layer formulation having the components described below in TABLES IV and V, using a bar coater to

provide a dry coating weight of radiation-sensitive imageable layer of 0.9 g/m<sup>2</sup> after drying at 50° C. for 60 seconds.

30

TABLE IV

| Components of Radiation-Sensitive Imageable Layer Formulation |                |
|---------------------------------------------------------------|----------------|
| Component                                                     | Amount (grams) |
| Polymer dispersion                                            | 0.747          |
| Hydroxypropyl methyl cellulose                                | 0.400          |
| Monomer 1                                                     | 0.333          |
| Monomer 2                                                     | 0.167          |
| IR dye 1                                                      | 0.020          |
| Leuco Dye 1                                                   | 0.023          |
| Surfactant 1                                                  | 0.045          |
| Iodonium salt                                                 | 0.05           |
| 1-Propanol                                                    | 3.27           |
| 2-Butanone                                                    | 1.60           |
| 1-Methoxy-2-propanol                                          | 2.82           |
| δ-Butyrolactone                                               | 0.10           |
| Water                                                         | 0.43           |

TABLE V

| Description of Certain Radiation-sensitive Imageable Layer Components |                                                                                                                                                                                            |
|-----------------------------------------------------------------------|--------------------------------------------------------------------------------------------------------------------------------------------------------------------------------------------|
| Polymer dispersion                                                    | The polymer dispersion prepared according to Example 10 of EP 1,765,593A1, used as 23.5 weight % polymer in n-propanol/water at 80:20 weight ratio                                         |
| Hydroxy propyl methyl cellulose                                       | 5 weight % hydroxypropyl methyl cellulose polymer in water; the polymer is 30% methoxylated, 10% hydroxyl propoxylated and has a viscosity of 5 mPa sec in a 2% aqueous solution at 20° C. |

TABLE V-continued

| Description of Certain Radiation-sensitive Imageable Layer Components |                                                                                                                                                                                                                                                                                                                                         |
|-----------------------------------------------------------------------|-----------------------------------------------------------------------------------------------------------------------------------------------------------------------------------------------------------------------------------------------------------------------------------------------------------------------------------------|
| Monomer 1                                                             | Urethane acrylate prepared by reacting DESMODUR ® N100 (from Bayer Corp., Milford, CT) with hydroxyethyl acrylate and pentaerythritol triacrylate at approximately 1:1.5:1.5 molar ratio (40 weight % in 2-butanone).                                                                                                                   |
| Monomer 2                                                             | Ethoxylated (10 EO) Bisphenol A acrylate, 40 weight % in 2-butanone                                                                                                                                                                                                                                                                     |
| IR dye 1                                                              | <p>Chemical structure of IR dye 1: A bis(4-phenyl-2-butene-1-yl) bis(2-mercapto-4-thiophenyl sulfide). It consists of two 4-phenyl-2-butene-1-yl groups connected by a central bis(2-mercapto-4-thiophenyl sulfide) bridge. The phenyl groups are substituted with a 4-phenyl-2-butene-1-yl group at the para position.</p>             |
| Leuco dye 1                                                           | <p>Chemical structure of Leuco dye 1: A complex polycyclic aromatic compound. It features a central core with an oxazoline ring fused to a benzene ring. The core is substituted with a 4-(dimethylamino)phenyl group and a 4-methylphenyl group. The structure is highly conjugated, with multiple benzene rings and oxygen atoms.</p> |
| Iodonium salt                                                         | A tetraphenyl borate salt having the following cation:                                                                                                                                                                                                                                                                                  |
|                                                                       | <p>Chemical structure of the cation of the Iodonium salt: A tetraphenyl borate cation. It consists of a central boron atom bonded to four phenyl groups (each with a methyl group at the para position) and an iodide (I<sup>-</sup>) counterion.</p>                                                                                   |
| Surfactant 1                                                          | BYK ® 302 from Byk Chemie, used as a 25 weight % solution in 1-methoxy-2-propanol                                                                                                                                                                                                                                                       |

Each of the Invention lithographic printing plate precursors was evaluated with respect to press life, on-press developability, and scratch resistance using the test methods described below and the results are shown in the following TABLE VI.

#### Press Life Evaluation:

To evaluate press life, each lithographic printing plate precursor was imagewise exposed using a Trendsetter 800 III Quantum (available from Eastman Kodak Company) at 150 mJ/cm<sup>2</sup> and then mounted on a FAVORIT 04 printing press (available from Man Roland) without any development process in between. In other words, each was developed on-press using the printing press that was operated with Vam Supreme 6038+Par fountain solution and Gans Cyan printing ink. The press life printing test was performed up to

100,000 impressions with each resulting lithographic printing plate. With ongoing printing, the lithographic printing plates were gradually abraded.

The “press life” for each lithographic printing plate is defined as the number of printed paper sheets before the tonal value of the printed paper sheets in a 50% FM20 screen had been reduced to 70% or less of the tonal value obtained on the 1000<sup>th</sup> sheet. For the measurement of tonal values, a Techkon Spectro Dens spectral densitometer was used, and the results were scored as follows:

A: equal to or more than 80,000 sheets

B: equal to or more than 60,000 sheets, but less than 80,000 sheets

C: equal to or more than 40,000 sheets, but less than 60,000 sheets

D: equal to or more than 12,000 sheets, but less than 40,000 sheets

E: less than 12,000 sheets

On-Press Developability:

On-press developability was evaluated under the same exposure and printing press conditions as for the press life test, but only the first 1000 printed sheets were evaluated for each lithographic printing plate, and each precursor was exposed in segments at different energies of between 50 mJ/cm<sup>2</sup> and 300 mJ/cm<sup>2</sup> instead of 150 mJ/cm<sup>2</sup> on the full printing plate. On the first 10 revolutions, the printing press was operated only with fountain solution, and afterwards lithographic ink was supplied to the lithographic printing plates and printing paper was fed to the machine. During the on-press development process, the non-exposed regions of the radiation-sensitive imageable layer initially transferred lithographic ink to printed sheets. On-press development was finished when the lithographic ink density on the printed sheets in the non-exposed regions (corresponding to the non-image regions) became invisible to the naked eye and was scored as follows:

A: development finished with 5 or fewer sheets of paper

B: development finished with more than 5 sheets, but 10 or fewer sheets of paper

C: development finished with more than 10 sheets, but 15 or fewer sheets of paper

D: development finished with more than 15 sheets, but 50 or fewer sheets of paper

E: development finished with more than 50 sheets of paper

Scratch Resistance:

To assess scratch resistance, a heavy duty scouring pad (marketed for household cleaning) was placed under a weight with a circular shape having a diameter of 50 mm, and pulled at a constant speed of 0.2 m/sec across the radiation-sensitive imageable layer side of each lithographic printing plate precursor cut into a rectangular shape of 600 mm×200 mm. The procedure was repeated on different regions of each lithographic printing plate precursor using weights that varied as 100 g, 300 g, 600 g, 900 g, and 1200 g. The precursors afterwards were dipped into a 100 ml CuSO<sub>4</sub> solution for 60 seconds at 20° C., in which the CuSO<sub>4</sub> reacted with the bare aluminum metal exposed in the scratches, rendering them a brownish color. The CuSO<sub>4</sub> solution was obtained by dissolving 151 g of CuSO<sub>4</sub>·5H<sub>2</sub>O in 800 ml of 1.0 molar HCl and then diluting the resulting solution with equal amount of deionized water. Each lithographic printing plate precursor treated in this manner was visually assessed and the total number of individual brownish scratches was determined, where 10 or less scratches in one run with one of the weights were recorded as the actual count and more than 10 scratches in one run with one of the weights were counted as "20". The following scoring method was used in the evaluation:

A: less than 30 scratches

B: equal to or more than 30 scratches but less than 40 scratches

C: equal to or more than 40 scratches but less than 50 scratches

D: equal to or more than 50 scratches but less than 70 scratches

E: equal to or more than 70 scratches

Edge Burn Tendency:

The edge burn tendency was tested optically, since differences in oxide layer thickness can easily be evaluated by eye due to color changes of the inventive substrate surface. The evaluation was scored as follows:

A: plate looks absolutely smooth and regular, no hint to edge burn

C: very slight irregularities on the plate (nearly invisible)

E: severe irregularities

TABLE VI

| Properties of Invention Precursors |                   |            |                         |                    |                    |
|------------------------------------|-------------------|------------|-------------------------|--------------------|--------------------|
|                                    | Invention Example | Press Life | On-press Developability | Scratch Resistance | Edge Burn Tendency |
| 10                                 | 1                 | B          | A                       | A                  | A                  |
|                                    | 2                 | B          | A                       | A                  | A                  |
|                                    | 3                 | A          | A                       | A                  | A                  |
| 15                                 | 4                 | A          | A                       | A                  | A                  |
|                                    | 5                 | A          | A                       | A                  | A                  |
|                                    | 6                 | C          | A                       | A                  | A                  |
|                                    | 7                 | B          | A                       | A                  | A                  |
|                                    | 8                 | A          | A                       | A                  | A                  |
|                                    | 9                 | A          | A                       | A                  | A                  |
| 20                                 | 10                | A          | A                       | A                  | A                  |
|                                    | 11                | C          | C                       | A                  | C                  |
|                                    | 12                | B          | C                       | A                  | C                  |
|                                    | 13                | B          | C                       | A                  | C                  |
|                                    | 14                | A          | C                       | A                  | C                  |
|                                    | 15                | B          | A                       | C                  | A                  |
|                                    | 16                | C          | A                       | C                  | A                  |
|                                    | 17                | B          | C                       | C                  | C                  |
|                                    | 18                | B          | A                       | A                  | A                  |
|                                    | 19                | A          | A                       | A                  | A                  |
|                                    | 20                | B          | A                       | A                  | A                  |
|                                    | 21                | C          | A                       | A                  | A                  |
| 30                                 | 22                | B          | C                       | A                  | C                  |
|                                    | 23                | B          | A                       | A                  | A                  |
|                                    | 24                | C          | A                       | A                  | A                  |
|                                    | 25                | B          | C                       | A                  | C                  |
|                                    | 28                | A          | A                       | A                  | A                  |
|                                    | 29                | A          | A                       | A                  | A                  |
|                                    | 30                | A          | A                       | A                  | A                  |
| 35                                 | 31                | A          | A                       | A                  | A                  |

The results shown above in TABLE VI show that the lithographic printing plate precursors of Invention Examples 1-31 exhibited excellent press life after imaging, on-press developability, and scratch resistance while showing no tendency to edge burn. Each inner aluminum oxide layer, having an average inner micropore diameter (D<sub>i</sub>) of less than 15 nm and an average dry thickness (T<sub>i</sub>) of at least 650 nm is believed to be responsible for the desired scratch resistance. It can be further seen that in general, the thicker of the inner aluminum oxide layer, the better the scratch resistance observed.

The excellent press life and on-press developability properties of the lithographic printing plate precursors of Invention Examples 1-31 are believed to be provided at least in part from the porous structure of the outer aluminum oxide layer that had an average outer micropore diameter (D<sub>o</sub>) of at least 15 nm and up to and including 30 nm, a porosity (P<sub>o</sub>) of at least 30% and up to and including 80%, and average dry thickness (T<sub>o</sub>) of at least 150 nm.

Comparative Examples 1 to 50

Comparative lithographic printing plate substrates and precursors labeled as Comparative Examples 1-51 were prepared in the same manner as described above for Invention Examples 1-31 except that the grained and etched substrates were anodized using the parameters described below in TABLE VII. For Comparative Examples 30-35, no second anodizing process was carried out. For Comparative Examples 41-50, a micropore-widening step was performed

after the first anodizing process and before a second anodizing process by etching the outer aluminum oxide layer with an alkaline solution.

In TABLE VII, the parameters are identified as follows:

A1=Electrolyte  
A2=Electrolyte concentration (g/liter)  
A3=Temperature (° C.)  
A4=Current density (A/dm<sup>2</sup>)  
A5=Time (seconds)  
A6=Charge density (C/dm<sup>2</sup>)

B1=Electrolyte  
B2=Electrolyte concentration (g/liter)  
B3=Temperature (° C.)  
B4=Time (seconds)  
5 C1=Electrolyte  
C2=Electrolyte concentration (g/liter)  
C3=Temperature (° C.)  
C4=Current density (A/dm<sup>2</sup>)  
C5=Time (seconds)  
C6=Charge density (C/dm<sup>2</sup>)

TABLE VII

| Comparative Example | Process Parameters for Substrate Preparation |     |    |      |       |       |                    |    |    |    |                                |     |    |      |      |       |
|---------------------|----------------------------------------------|-----|----|------|-------|-------|--------------------|----|----|----|--------------------------------|-----|----|------|------|-------|
|                     | First Anodizing Process                      |     |    |      |       |       | Micropore Widening |    |    |    | Second Anodizing Process       |     |    |      |      |       |
|                     | A1                                           | A2  | A3 | A4   | A5    | A6    | B1                 | B2 | B3 | B4 | C1                             | C2  | C3 | C4   | C5   | C6    |
| 1                   | H <sub>3</sub> PO <sub>4</sub>               | 300 | 60 | 8.5  | 1.6   | 13.8  |                    |    |    |    | H <sub>2</sub> SO <sub>4</sub> | 280 | 23 | 10.0 | 18.0 | 180.0 |
| 2                   | H <sub>3</sub> PO <sub>4</sub>               | 250 | 60 | 6.6  | 4.2   | 27.6  |                    |    |    |    | H <sub>2</sub> SO <sub>4</sub> | 280 | 23 | 10.0 | 18.0 | 180.0 |
| 3                   | H <sub>3</sub> PO <sub>4</sub>               | 200 | 60 | 5.5  | 8.0   | 44.2  |                    |    |    |    | H <sub>2</sub> SO <sub>4</sub> | 280 | 23 | 10.0 | 18.0 | 180.0 |
| 4                   | H <sub>3</sub> PO <sub>4</sub>               | 175 | 50 | 1.8  | 7.7   | 13.8  |                    |    |    |    | H <sub>2</sub> SO <sub>4</sub> | 280 | 23 | 10.0 | 18.0 | 180.0 |
| 5                   | H <sub>3</sub> PO <sub>4</sub>               | 175 | 55 | 3.8  | 7.3   | 27.6  |                    |    |    |    | H <sub>2</sub> SO <sub>4</sub> | 280 | 23 | 10.0 | 18.0 | 180.0 |
| 6                   | H <sub>3</sub> PO <sub>4</sub>               | 100 | 50 | 3.3  | 4.2   | 13.8  |                    |    |    |    | H <sub>2</sub> SO <sub>4</sub> | 280 | 23 | 10.0 | 18.0 | 180.0 |
| 7                   | H <sub>3</sub> PO <sub>4</sub>               | 150 | 50 | 5.2  | 5.4   | 27.6  |                    |    |    |    | H <sub>2</sub> SO <sub>4</sub> | 280 | 23 | 10.0 | 18.0 | 180.0 |
| 8                   | H <sub>3</sub> PO <sub>4</sub>               | 200 | 50 | 7.1  | 6.3   | 44.2  |                    |    |    |    | H <sub>2</sub> SO <sub>4</sub> | 280 | 23 | 10.0 | 18.0 | 180.0 |
| 9                   | H <sub>3</sub> PO <sub>4</sub>               | 50  | 60 | 18.6 | 0.7   | 13.8  |                    |    |    |    | H <sub>2</sub> SO <sub>4</sub> | 280 | 23 | 10.0 | 18.0 | 180.0 |
| 10                  | H <sub>3</sub> PO <sub>4</sub>               | 100 | 60 | 20.5 | 1.3   | 27.6  |                    |    |    |    | H <sub>2</sub> SO <sub>4</sub> | 280 | 23 | 10.0 | 18.0 | 180.0 |
| 11                  | H <sub>3</sub> PO <sub>4</sub>               | 150 | 60 | 22.4 | 2.0   | 44.2  |                    |    |    |    | H <sub>2</sub> SO <sub>4</sub> | 280 | 23 | 10.0 | 18.0 | 180.0 |
| 12                  | H <sub>3</sub> PO <sub>4</sub>               | 200 | 60 | 24.3 | 2.9   | 70.7  |                    |    |    |    | H <sub>2</sub> SO <sub>4</sub> | 280 | 23 | 10.0 | 18.0 | 180.0 |
| 13                  | H <sub>3</sub> PO <sub>4</sub>               | 250 | 60 | 26.2 | 4.7   | 123.7 |                    |    |    |    | H <sub>2</sub> SO <sub>4</sub> | 280 | 23 | 10.0 | 18.0 | 180.0 |
| 14                  | H <sub>3</sub> PO <sub>4</sub>               | 300 | 60 | 28.1 | 6.3   | 176.7 |                    |    |    |    | H <sub>2</sub> SO <sub>4</sub> | 280 | 23 | 10.0 | 18.0 | 180.0 |
| 15                  | H <sub>3</sub> PO <sub>4</sub>               | 350 | 60 | 30.0 | 9.6   | 287.6 |                    |    |    |    | H <sub>2</sub> SO <sub>4</sub> | 280 | 23 | 10.0 | 18.0 | 180.0 |
| 16                  | H <sub>3</sub> PO <sub>4</sub>               | 150 | 60 | 22.4 | 18.8  | 419.3 |                    |    |    |    | H <sub>2</sub> SO <sub>4</sub> | 280 | 23 | 10.0 | 18.0 | 180.0 |
| 17                  | H <sub>3</sub> PO <sub>4</sub>               | 150 | 55 | 1.8  | 53.6  | 123.6 |                    |    |    |    | H <sub>2</sub> SO <sub>4</sub> | 280 | 23 | 10.0 | 6.8  | 67.5  |
| 18                  | H <sub>3</sub> PO <sub>4</sub>               | 150 | 55 | 2.9  | 12.8  | 44.0  |                    |    |    |    | H <sub>2</sub> SO <sub>4</sub> | 280 | 23 | 10.0 | 6.8  | 67.5  |
| 19                  | H <sub>3</sub> PO <sub>4</sub>               | 150 | 55 | 7.1  | 23.1  | 177.7 |                    |    |    |    | H <sub>2</sub> SO <sub>4</sub> | 280 | 23 | 10.0 | 6.8  | 67.5  |
| 20                  | H <sub>3</sub> PO <sub>4</sub>               | 150 | 55 | 20.3 | 3.5   | 67.1  |                    |    |    |    | H <sub>2</sub> SO <sub>4</sub> | 280 | 23 | 10.0 | 6.8  | 67.5  |
| 21                  | H <sub>3</sub> PO <sub>4</sub>               | 250 | 55 | 5.6  | 53.8  | 123.7 |                    |    |    |    | H <sub>2</sub> SO <sub>4</sub> | 280 | 23 | 10.0 | 11.3 | 112.5 |
| 22                  | H <sub>3</sub> PO <sub>4</sub>               | 250 | 55 | 6.7  | 13.0  | 44.2  |                    |    |    |    | H <sub>2</sub> SO <sub>4</sub> | 280 | 23 | 10.0 | 11.3 | 112.5 |
| 23                  | H <sub>3</sub> PO <sub>4</sub>               | 250 | 55 | 10.9 | 23.1  | 176.7 |                    |    |    |    | H <sub>2</sub> SO <sub>4</sub> | 280 | 23 | 10.0 | 11.3 | 112.5 |
| 24                  | H <sub>3</sub> PO <sub>4</sub>               | 250 | 55 | 24.1 | 3.4   | 70.7  |                    |    |    |    | H <sub>2</sub> SO <sub>4</sub> | 280 | 23 | 10.0 | 11.3 | 112.5 |
| 25                  | H <sub>3</sub> PO <sub>4</sub>               | 350 | 55 | 27.9 | 3.5   | 66.9  |                    |    |    |    | H <sub>2</sub> SO <sub>4</sub> | 280 | 23 | 10.0 | 15.0 | 150.0 |
| 26                  | H <sub>3</sub> PO <sub>4</sub>               | 250 | 55 | 10.9 | 5.8   | 44.2  |                    |    |    |    | H <sub>2</sub> SO <sub>4</sub> | 280 | 23 | 10.0 | 33.8 | 337.5 |
| 27                  | H <sub>3</sub> PO <sub>4</sub>               | 250 | 55 | 24.1 | 5.9   | 123.7 |                    |    |    |    | H <sub>2</sub> SO <sub>4</sub> | 280 | 23 | 10.0 | 33.8 | 337.5 |
| 28                  | H <sub>3</sub> PO <sub>4</sub>               | 150 | 55 | 20.3 | 3.5   | 73.4  |                    |    |    |    | H <sub>2</sub> SO <sub>4</sub> | 280 | 23 | 10.0 | 45.0 | 450.0 |
| 29                  | H <sub>3</sub> PO <sub>4</sub>               | 350 | 55 | 27.9 | 3.4   | 71.9  |                    |    |    |    | H <sub>2</sub> SO <sub>4</sub> | 280 | 23 | 10.0 | 67.5 | 675.0 |
| 30                  | H <sub>3</sub> PO <sub>4</sub>               | 175 | 55 | 3.5  | 19.2  | 67.1  |                    |    |    |    |                                |     |    |      |      | 0.0   |
| 31                  | H <sub>3</sub> PO <sub>4</sub>               | 175 | 55 | 3.5  | 41.7  | 145.9 |                    |    |    |    |                                |     |    |      |      | 0.0   |
| 32                  | H <sub>3</sub> PO <sub>4</sub>               | 175 | 55 | 3.5  | 62.7  | 219.4 |                    |    |    |    |                                |     |    |      |      | 0.0   |
| 33                  | H <sub>3</sub> PO <sub>4</sub>               | 175 | 55 | 3.5  | 80.4  | 281.3 |                    |    |    |    |                                |     |    |      |      | 0.0   |
| 34                  | H <sub>3</sub> PO <sub>4</sub>               | 175 | 55 | 3.5  | 96.5  | 337.8 |                    |    |    |    |                                |     |    |      |      | 0.0   |
| 35                  | H <sub>3</sub> PO <sub>4</sub>               | 175 | 55 | 3.5  | 188.1 | 658.3 |                    |    |    |    |                                |     |    |      |      | 0.0   |
| 36                  | H <sub>2</sub> SO <sub>4</sub>               | 280 | 23 | 10.0 | 11.3  | 112.5 |                    |    |    |    | H <sub>2</sub> SO <sub>4</sub> | 280 | 23 | 10.0 | 18.0 | 180.0 |
| 37                  | H <sub>2</sub> SO <sub>4</sub>               | 280 | 23 | 16.0 | 8.4   | 135.0 |                    |    |    |    | H <sub>2</sub> SO <sub>4</sub> | 280 | 23 | 10.0 | 18.0 | 180.0 |
| 38                  | H <sub>2</sub> SO <sub>4</sub>               | 280 | 23 | 24.0 | 6.7   | 160.0 |                    |    |    |    | H <sub>2</sub> SO <sub>4</sub> | 280 | 23 | 10.0 | 18.0 | 180.0 |
| 39                  | H <sub>2</sub> SO <sub>4</sub>               | 280 | 23 | 30.0 | 5.3   | 160.0 |                    |    |    |    | H <sub>2</sub> SO <sub>4</sub> | 280 | 23 | 10.0 | 18.0 | 180.0 |
| 40                  | H <sub>2</sub> SO <sub>4</sub>               | 280 | 23 | 45.0 | 3.6   | 160.0 |                    |    |    |    | H <sub>2</sub> SO <sub>4</sub> | 280 | 23 | 10.0 | 18.0 | 180.0 |
| 41                  | H <sub>2</sub> SO <sub>4</sub>               | 280 | 23 | 10.0 | 1.4   | 13.5  | NaOH               | 5  | 35 | 1  | H <sub>2</sub> SO <sub>4</sub> | 280 | 23 | 10.0 | 18.0 | 180.0 |
| 42                  | H <sub>2</sub> SO <sub>4</sub>               | 280 | 23 | 10.0 | 1.4   | 13.5  | NaOH               | 5  | 35 | 4  | H <sub>2</sub> SO <sub>4</sub> | 280 | 23 | 10.0 | 18.0 | 180.0 |
| 43                  | H <sub>2</sub> SO <sub>4</sub>               | 280 | 23 | 10.0 | 1.4   | 13.5  | NaOH               | 5  | 35 | 6  | H <sub>2</sub> SO <sub>4</sub> | 280 | 23 | 10.0 | 18.0 | 180.0 |
| 44                  | H <sub>2</sub> SO <sub>4</sub>               | 280 | 23 | 10.0 | 1.4   | 13.5  | NaOH               | 5  | 35 | 12 | H <sub>2</sub> SO <sub>4</sub> | 280 | 23 | 10.0 | 18.0 | 180.0 |
| 45                  | H <sub>2</sub> SO <sub>4</sub>               | 280 | 23 | 10.0 | 1.4   | 13.5  | NaOH               | 5  | 35 | 20 | H <sub>2</sub> SO <sub>4</sub> | 280 | 23 | 10.0 | 18.0 | 180.0 |
| 46                  | H <sub>2</sub> SO <sub>4</sub>               | 280 | 23 | 10.0 | 2.5   | 25.0  | NaOH               | 5  | 35 | 6  | H <sub>2</sub> SO <sub>4</sub> | 280 | 23 | 10.0 | 18.0 | 180.0 |
| 47                  | H <sub>2</sub> SO <sub>4</sub>               | 280 | 23 | 10.0 | 7.6   | 76.0  | NaOH               | 5  | 35 | 6  | H <sub>2</sub> SO <sub>4</sub> | 280 | 23 | 10.0 | 18.0 | 180.0 |
| 48                  | H <sub>2</sub> SO <sub>4</sub>               | 170 | 43 | 30.0 | 1.0   | 30.0  | NaOH               | 5  | 35 | 6  | H <sub>2</sub> SO <sub>4</sub> | 170 | 43 | 15.0 | 14.7 | 220.0 |
| 49                  | H <sub>2</sub> SO <sub>4</sub>               | 170 | 43 | 30.0 | 1.0   | 30.0  | NaOH               | 5  | 35 | 4  | H <sub>2</sub> SO <sub>4</sub> | 170 | 40 | 20.0 | 12.5 | 250.0 |
| 50                  | H <sub>2</sub> SO <sub>4</sub>               | 170 | 43 | 50.0 | 1.0   | 50.0  | NaOH               | 5  | 35 | 16 | H <sub>2</sub> SO <sub>4</sub> | 170 | 40 | 20.0 | 12.5 | 250.0 |

The lithographic printing plate substrates prepared for Comparative Examples 1-50 were evaluated using the same techniques as applied above for evaluating the inventive substrates of Invention Examples 1-31 and the determined structural features are shown in the following TABLE VIII.

TABLE VIII

| Comparative Example | Outer Aluminum Oxide Layer                   |                                                   |                                                          |                                | Inner Aluminum Oxide Layer                   |                                                   |     |
|---------------------|----------------------------------------------|---------------------------------------------------|----------------------------------------------------------|--------------------------------|----------------------------------------------|---------------------------------------------------|-----|
|                     | Average Dry Thickness (T <sub>o</sub> ) [nm] | Average Micropore Diameter (D <sub>o</sub> ) [nm] | Micropore Density (C <sub>o</sub> ) [1/μm <sup>2</sup> ] | Porosity (P <sub>o</sub> ) [%] | Average Dry Thickness (T <sub>i</sub> ) [nm] | Average Micropore Diameter (D <sub>i</sub> ) [nm] |     |
|                     | 1                                            | 43                                                | 19                                                       | 2703                           | 76                                           | 785                                               | <10 |
| 2                   | 77                                           | 19                                                | 2854                                                     | 81                             | 774                                          | <10                                               |     |
| 3                   | 128                                          | 17                                                | 2736                                                     | 64                             | 821                                          | <10                                               |     |
| 4                   | 39                                           | 20                                                | 1312                                                     | 40                             | 799                                          | <10                                               |     |
| 5                   | 78                                           | 22                                                | 1343                                                     | 52                             | 804                                          | <10                                               |     |
| 6                   | 53                                           | 29                                                | 582                                                      | 39                             | 816                                          | <10                                               |     |
| 7                   | 94                                           | 29                                                | 592                                                      | 39                             | 787                                          | <10                                               |     |
| 8                   | 140                                          | 31                                                | 626                                                      | 47                             | 773                                          | <10                                               |     |
| 9                   | 41                                           | 36                                                | 380                                                      | 39                             | 788                                          | <10                                               |     |
| 10                  | 92                                           | 36                                                | 372                                                      | 38                             | 811                                          | <10                                               |     |
| 11                  | 185                                          | 38                                                | 376                                                      | 42                             | 830                                          | <10                                               |     |
| 12                  | 215                                          | 34                                                | 367                                                      | 33                             | 797                                          | <10                                               |     |
| 13                  | 312                                          | 39                                                | 370                                                      | 44                             | 807                                          | <10                                               |     |
| 14                  | 348                                          | 36                                                | 392                                                      | 40                             | 820                                          | <10                                               |     |
| 15                  | 489                                          | 37                                                | 383                                                      | 40                             | 808                                          | <10                                               |     |
| 16                  | 587                                          | 39                                                | 381                                                      | 46                             | 775                                          | <10                                               |     |
| 17                  | 311                                          | 17                                                | 2703                                                     | 64                             | 287                                          | <10                                               |     |
| 18                  | 146                                          | 22                                                | 1308                                                     | 51                             | 299                                          | <10                                               |     |
| 19                  | 479                                          | 27                                                | 628                                                      | 36                             | 288                                          | <10                                               |     |
| 20                  | 213                                          | 34                                                | 386                                                      | 35                             | 295                                          | <10                                               |     |
| 21                  | 311                                          | 16                                                | 2610                                                     | 55                             | 517                                          | <10                                               |     |
| 22                  | 142                                          | 20                                                | 1222                                                     | 37                             | 508                                          | <10                                               |     |
| 23                  | 503                                          | 27                                                | 580                                                      | 33                             | 528                                          | <10                                               |     |
| 24                  | 207                                          | 35                                                | 385                                                      | 36                             | 494                                          | <10                                               |     |
| 25                  | 224                                          | 33                                                | 375                                                      | 32                             | 623                                          | <10                                               |     |
| 26                  | 163                                          | 32                                                | 619                                                      | 50                             | 1508                                         | <10                                               |     |
| 27                  | 305                                          | 38                                                | 377                                                      | 44                             | 1519                                         | <10                                               |     |
| 28                  | 183                                          | 36                                                | 395                                                      | 41                             | 2023                                         | <10                                               |     |
| 29                  | 191                                          | 36                                                | 376                                                      | 39                             | 3028                                         | <10                                               |     |
| 30                  | 190                                          | 21                                                | 1311                                                     | 47                             | 0                                            | NA-1                                              |     |
| 31                  | 413                                          | 22                                                | 1316                                                     | 50                             | 0                                            | NA-1                                              |     |
| 32                  | 621                                          | 20                                                | 1234                                                     | 38                             | 0                                            | NA-1                                              |     |
| 33                  | 796                                          | 19                                                | 1227                                                     | 37                             | 0                                            | NA-1                                              |     |
| 34                  | 956                                          | 22                                                | 1222                                                     | 47                             | 0                                            | NA-1                                              |     |
| 35                  | 1863                                         | 23                                                | 1338                                                     | 55                             | 0                                            | NA-1                                              |     |
| 36                  | 512                                          | <10                                               | NA-2                                                     | NA-2                           | 804                                          | <10                                               |     |
| 37                  | 615                                          | <10                                               | NA-2                                                     | NA-2                           | 790                                          | <10                                               |     |
| 38                  | 681                                          | <10                                               | NA-2                                                     | NA-2                           | 797                                          | <10                                               |     |
| 39                  | 703                                          | <10                                               | NA-2                                                     | NA-2                           | 778                                          | <10                                               |     |
| 40                  | 719                                          | <10                                               | NA-2                                                     | NA-2                           | 773                                          | <10                                               |     |
| 41                  | 60                                           | <10                                               | 2430                                                     | <21                            | 809                                          | <10                                               |     |
| 42                  | 62                                           | <10                                               | 2613                                                     | <21                            | 788                                          | <10                                               |     |
| 43                  | 62                                           | 10                                                | 2575                                                     | 20                             | 796                                          | <10                                               |     |
| 44                  | 61                                           | 13                                                | 2501                                                     | 33                             | 793                                          | <10                                               |     |
| 45                  | 62                                           | NA-3                                              | NA-3                                                     | 90-100                         | 817                                          | <10                                               |     |
| 46                  | 114                                          | 13                                                | 2567                                                     | 34                             | 801                                          | <10                                               |     |
| 47                  | 336                                          | 13                                                | 2468                                                     | 33                             | 792                                          | <10                                               |     |
| 48                  | 47                                           | 25                                                | 553                                                      | 27                             | 926                                          | <10                                               |     |
| 49                  | 45                                           | 21                                                | 623                                                      | 22                             | 985                                          | <10                                               |     |
| 50                  | 79                                           | 48                                                | 472                                                      | 85                             | 1012                                         | <10                                               |     |

NA-1: not applicable due to absence of the inner aluminum oxide layer;

NA-2: the micropore diameter in the outer aluminum oxide layer is too small to measure micropore density and to calculate the porosity;

NA-3: the outer aluminum oxide layer was severely damaged by the micropore-widening treatment such that it was not possible to measure the micropore diameter and micropore density.

Comparative Examples 1-50 lithographic printing plate precursors were prepared using the corresponding substrates described above by applying the hydrophilic layer formulation and negative-working radiation-sensitive imageable layer formulation described above for Invention Examples

1-31. The resulting lithographic printing plate precursors were imagewise exposed (when appropriate) and evaluated using the same procedures and evaluation tests as described above for Invention Examples 1-31. The results of these evaluations are shown in the following TABLE IX.

TABLE IX

| Properties of Comparative Precursors |            |                         |                    |                    |
|--------------------------------------|------------|-------------------------|--------------------|--------------------|
| Comparative Example                  | Press Life | On-press Developability | Scratch Resistance | Edge Burn Tendency |
| 1                                    | E          | A                       | A                  | A                  |
| 2                                    | D          | A                       | A                  | A                  |
| 3                                    | C          | A                       | A                  | A                  |
| 4                                    | E          | A                       | A                  | A                  |
| 5                                    | D          | A                       | A                  | A                  |
| 6                                    | E          | C                       | A                  | C                  |
| 7                                    | E          | C                       | A                  | C                  |
| 8                                    | C          | D                       | A                  | C                  |
| 9                                    | E          | D                       | A                  | E                  |
| 10                                   | E          | D                       | A                  | E                  |
| 11                                   | D          | D                       | A                  | E                  |
| 12                                   | D          | D                       | A                  | E                  |
| 13                                   | D          | D                       | A                  | E                  |
| 14                                   | C          | D                       | A                  | E                  |
| 15                                   | B          | D                       | A                  | E                  |
| 16                                   | A          | D                       | A                  | E                  |
| 17                                   | B          | A                       | D                  | A                  |
| 18                                   | B          | A                       | D                  | A                  |
| 19                                   | B          | C                       | D                  | C                  |
| 20                                   | D          | D                       | D                  | E                  |
| 21                                   | B          | A                       | D                  | A                  |
| 22                                   | C          | A                       | D                  | A                  |
| 23                                   | B          | C                       | D                  | C                  |
| 24                                   | D          | D                       | D                  | E                  |
| 25                                   | D          | D                       | C                  | E                  |
| 26                                   | D          | C                       | A                  | C                  |
| 27                                   | D          | D                       | A                  | E                  |
| 28                                   | D          | D                       | A                  | E                  |
| 29                                   | D          | D                       | A                  | E                  |
| 30                                   | B          | A                       | E                  | A                  |
| 31                                   | A          | A                       | E                  | A                  |
| 32                                   | A          | A                       | E                  | A                  |
| 33                                   | A          | A                       | D                  | A                  |
| 34                                   | A          | A                       | D                  | A                  |
| 35                                   | A          | A                       | D                  | A                  |
| 36                                   | E          | E                       | A                  | A                  |
| 37                                   | E          | E                       | A                  | A                  |
| 38                                   | E          | E                       | A                  | A                  |
| 39                                   | E          | E                       | A                  | C                  |
| 40                                   | E          | E                       | A                  | D                  |
| 41                                   | E          | E                       | A                  | A                  |
| 42                                   | E          | E                       | A                  | A                  |
| 43                                   | E          | E                       | A                  | A                  |
| 44                                   | E          | E                       | A                  | A                  |
| 45                                   | E          | E                       | A                  | A                  |
| 46                                   | E          | E                       | A                  | A                  |
| 47                                   | E          | E                       | A                  | A                  |
| 48                                   | E          | E                       | A                  | A                  |
| 49                                   | E          | E                       | A                  | A                  |
| 50                                   | E          | E                       | A                  | A                  |

The results shown in TABLE IX for Comparative Examples 1-50 that are outside of the present invention reveal one or more disadvantages for each Comparative precursor over the results obtained from the Invention Examples 1-31 comprising inventive substrates. The precursors identified as Comparative Examples 17-25 showed unsatisfactory scratch resistance. These precursors were derived using substrates having an inner aluminum oxide layer with very small average inner micropore diameter ( $D_i$ ) ( $<10$  nm) and an average dry thickness ( $T_i$ ) of less than 650 nm. In Comparative Examples 30-35, the scratch resistance was inadequate because the inner aluminum oxide layer was not formed. Apparently, the omission of the inner aluminum oxide layer cannot be compensated for by increasing the average dry thickness ( $T_i$ ) of the outer aluminum oxide layer. The average outer micropore diameter ( $D_o$ ) of the outer aluminum oxide layer is important for the on-press developability of the imagewise exposed precursor. If the

average outer micropore diameter ( $D_o$ ) is too small, as in the substrates of Comparative Examples 36-40, or too large as in the substrates used in Comparative Examples 8-16, 20, 24-29, and 50, on-press-developability of the imagewise exposed precursor is inadequate. Moreover, the precursor press life is low when the average dry layer thickness ( $T_o$ ) of the outer aluminum oxide layer is too small as in the case of the substrates used in Comparative Examples 1-7, 9, 10, 41-46, and 48-50.

In Comparative Examples 41-50, the micropores of the outer aluminum oxide layer were enlarged in a micropore widening step using a sodium hydroxide solution and procedures like those described in U.S. Pat. No. 8,783,179B2 (Kurokawa et al.), and EP Patent Publications 2,878,452A1 (Tagawa et al.) and 2,808,173A1 (Namba et al.), and an inner aluminum oxide layer was then formed underneath the outer aluminum oxide layer. For Comparative Example 45, a nearly complete dissolution of the outer aluminum oxide layer occurred during the micropore widening step. In general, the Comparative Examples in which a micropore widening process was used between the separate anodizing processes did not show adequate press life or on-press-developability. These Comparative Examples are outside the scope of the present invention due to the undesirable average outer micropore diameter, dry outer layer thickness, or outer aluminum oxide layer porosity.

The invention has been described in detail with particular reference to certain preferred embodiments thereof, but it will be understood that variations and modifications can be effected within the spirit and scope of the invention.

The invention claimed is:

1. A lithographic printing plate precursor comprising:  
a substrate having a planar surface, and  
a radiation-sensitive imageable layer disposed over the  
planar surface of the substrate,  
wherein the substrate comprises:

an aluminum-containing plate having a grained and  
etched planar surface;  
an inner aluminum oxide layer disposed on the grained  
and etched planar surface, the inner aluminum oxide  
layer: having an average dry thickness ( $T_i$ ) of at least  
650 nm and up to and including 3,000 nm; and com-  
prising a multiplicity of inner micropores having an  
average inner micropore diameter ( $D_i$ ) of less than or  
equal to 15 nm;

an outer aluminum oxide layer disposed on the inner  
aluminum oxide layer, the outer aluminum oxide layer:  
comprising a multiplicity of outer micropores having  
an average outer micropore diameter ( $D_o$ ) of at least 15  
nm and up to and including 30 nm; having an average  
dry thickness ( $T_o$ ) of at least 130 nm and up to and  
including 650 nm; and having a micropore density ( $C_o$ )  
of at least 500 micropores/ $\mu\text{m}^2$  and up to and including  
3,000 micropores/ $\mu\text{m}^2$ , wherein the ratio of the average  
outer micropore diameter ( $D_o$ ) to the average inner  
micropore diameter ( $D_i$ ) is greater than 1.1:1, and the  
average outer micropore diameter ( $D_o$ ) in nanometers  
and the micropore density ( $C_o$ ) in micropores/ $\mu\text{m}^2$ , are  
further constrained by the porosity ( $P_o$ ) of the outer  
aluminum oxide layer according to the following equa-  
tion:

$$0.3 \leq P_o \leq 0.8$$

wherein  $P_o$  is defined as  $3.14(C_o)(D_o^2)/4,000,000$ ; and  
optionally a hydrophilic layer comprising one or more  
hydrophilic polymers, which hydrophilic layer is dis-

posed on the outer aluminum oxide layer at a dry coverage of at least 0.0002 g/m<sup>2</sup> and up to and including 0.1 g/m<sup>2</sup>.

2. The lithographic printing plate precursor of claim 1, wherein the outer aluminum oxide layer has an average dry thickness (T<sub>o</sub>) of at least 150 nm and up to and including 400 nm.

3. The lithographic printing plate precursor of claim 1, wherein the inner aluminum oxide layer has an average dry thickness (T<sub>i</sub>) of at least 700 nm and up to and including 1500 nm.

4. The lithographic printing plate precursor of claim 1, wherein the following equation holds:

$$0.3 \leq P_o \leq 0.6.$$

5. The lithographic printing plate precursor of claim 1, wherein the ratio of the average outer micropore diameter (D<sub>o</sub>) to the average inner micropore diameter (D<sub>i</sub>) is at least 1.5:1.

6. The lithographic printing plate precursor of claim 1, further comprising the hydrophilic layer that comprises one or more water-soluble polymers, at least one of which water-soluble polymers comprises recurring units derived from either acrylic acid or methacrylic acid, or both acrylic acid and methacrylic acid.

7. The lithographic printing plate precursor of claim 1, wherein the radiation-sensitive imageable layer is sensitive to infrared radiation and comprises one or more infrared radiation absorbers.

8. The lithographic printing plate precursor of claim 1, wherein the radiation-sensitive imageable layer is positive-working and comprises one or more alkali-soluble polymers that are removable from the substrate upon exposure to radiation.

9. The lithographic printing plate precursor of claim 1, wherein the radiation-sensitive imageable layer is negative-working and comprises:

- (a) one or more free radically polymerizable components;
- (b) an initiator composition that provides free radicals upon exposure of the radiation-sensitive imageable layer to radiation;
- (c) one or more radiation absorbers; and optionally,
- (d) a polymeric binder that is different from all of (a), (b), and (c).

10. The lithographic printing plate precursor of claim 9, wherein the radiation-sensitive imageable layer is infrared

radiation-sensitive and the one or more radiation absorbers comprise one or more infrared radiation absorbers.

11. The lithographic printing plate precursor of claim 9, wherein the radiation-sensitive layer is negative-working and is on-press developable.

12. The lithographic printing plate precursor of claim 1 that is negative-working and further comprises a hydrophilic overcoat disposed over the radiation-sensitive imageable layer.

13. The lithographic printing plate precursor of claim 1, wherein:

the grained and etched planar surface of the aluminum-containing plate has been electrochemically grained and etched;

the hydrophilic layer is present and disposed on the outer aluminum oxide layer at a dry coverage of at least 0.005 g/m<sup>2</sup> and up to and including 0.08 g/m<sup>2</sup>, which hydrophilic layer comprises one or more hydrophilic polymers comprising recurring units derived at least in part from acrylic acid or methacrylic acid, or both; the radiation-sensitive imageable layer is a negative-working and on-press developable infrared radiation-sensitive imageable layer that is disposed on the hydrophilic layer:

- (a) one or more free radically polymerizable components;
- (b) an initiator composition that provides free radicals upon exposure of the radiation-sensitive imageable layer to infrared radiation;
- (c) one or more infrared radiation absorbers; and
- (d) a particulate polymeric binder that is different from all of (a), (b), and (c);

the inner aluminum oxide layer has an average dry thickness (T<sub>i</sub>) of at least 700 nm and up to and including 1,500 nm;

the outer aluminum oxide layer has an average dry thickness (T<sub>o</sub>) of at least 150 nm and up to and including 400 nm; and the ratio of the average outer micropore diameter (D<sub>o</sub>) to the average inner micropore diameter (D<sub>i</sub>) is at least 1.5:1 and the following equation holds:

$$0.3 \leq P_o \leq 0.6.$$

\* \* \* \* \*